



US010399206B1

(12) **United States Patent**  
**Mortensen et al.**

(10) **Patent No.:** **US 10,399,206 B1**  
(45) **Date of Patent:** **Sep. 3, 2019**

(54) **POLYCRYSTALLINE DIAMOND  
COMPACTS, METHODS OF FABRICATING  
THE SAME, AND METHODS OF USING THE  
SAME**

(71) Applicant: **US SYNTHETIC CORPORATION**,  
Orem, UT (US)

(72) Inventors: **Daniel Call Mortensen**, Eagle  
Mountain, UT (US); **Lindsay Sue  
Patton**, Provo, UT (US); **Trevor Allen  
Olsen**, Spanish Fork, UT (US); **Casey  
Wade Swan**, Spanish Fork, UT (US);  
**Shawn Casey Scott**, Payson, UT (US);  
**Matthew Kimball Baker**, Provo, UT  
(US); **Anne-Grethe Slotnaes**, South  
Jordan, UT (US); **Kenneth E.  
Bertagnoli**, Riverton, UT (US); **Jiang  
Qian**, Cedar Hills, UT (US); **Jason  
Lott**, Payson, UT (US); **Joshua Adam  
Hawks**, Saratoga Springs, UT (US)

(73) Assignee: **US SYNTHETIC CORPORATION**,  
Orem, UT (US)

(\*) Notice: Subject to any disclaimer, the term of this  
patent is extended or adjusted under 35  
U.S.C. 154(b) by 193 days.

(21) Appl. No.: **15/402,525**

(22) Filed: **Jan. 10, 2017**

**Related U.S. Application Data**

(60) Provisional application No. 62/279,271, filed on Jan.  
15, 2016.

(51) **Int. Cl.**  
**E21B 10/62** (2006.01)  
**E21B 10/633** (2006.01)  
(Continued)

(52) **U.S. Cl.**  
CPC ..... **B24D 3/007** (2013.01); **B24D 3/10**  
(2013.01); **E21B 10/55** (2013.01);  
(Continued)

(58) **Field of Classification Search**  
CPC ..... E21B 10/62; E21B 2010/622; E21B  
2010/624; E21B 10/633; E21B 10/567;  
(Continued)

(56) **References Cited**

**U.S. PATENT DOCUMENTS**

3,090,614 A 5/1963 Freeman et al.  
3,655,233 A 4/1972 Twist  
(Continued)

**FOREIGN PATENT DOCUMENTS**

WO 2016/044136 3/2016

**OTHER PUBLICATIONS**

U.S. Appl. No. 12/830,878, filed Jul. 6, 2010, Wiggins et al.  
(Continued)

*Primary Examiner* — Cathleen R Hutchins

(74) *Attorney, Agent, or Firm* — Dorsey & Whitney LLP

(57) **ABSTRACT**

PDCs, methods of fabricating the PDCs, and methods of using the PDCs are disclosed herein. The PDCs include a PCD table bonded to a substrate. The PCD table includes an upper surface having a plurality of recessed features formed therein. The plurality of recessed features are configured to attract at least some cracks that form in the PCD table. As such, the plurality of recessed features limit or prevent crack propagation into other portions of the PCD table and limit a volume of the PCD table that spalls. Methods of fabricating the PDCs include partially leaching the PCD table and, after leaching the PCD table, forming the plurality of recessed features in the upper surface thereof. Method of using the PDCs include rotating a PDC that has spalled relative to a rotary drill bit such that a portion of the upper surface of the PDC that has not spalled forms a cutting surface thereof.

**16 Claims, 25 Drawing Sheets**



|      |                                       |                                                                                          |                  |         |                     |              |
|------|---------------------------------------|------------------------------------------------------------------------------------------|------------------|---------|---------------------|--------------|
| (51) | <b>Int. Cl.</b>                       |                                                                                          |                  |         |                     |              |
|      | <i>E21B 10/567</i>                    | (2006.01)                                                                                | 8,950,519 B2     | 2/2015  | Gonzalez et al.     |              |
|      | <i>E21B 10/55</i>                     | (2006.01)                                                                                | 9,062,505 B2     | 6/2015  | Chapman et al.      |              |
|      | <i>B24D 3/00</i>                      | (2006.01)                                                                                | 9,175,521 B2     | 11/2015 | Bellin              |              |
|      | <i>B24D 3/10</i>                      | (2006.01)                                                                                | 9,260,923 B1     | 2/2016  | Bertagnolli et al.  |              |
| (52) | <b>U.S. Cl.</b>                       |                                                                                          | 9,610,555 B2     | 4/2017  | Mukhopadhyay et al. |              |
|      | CPC .....                             | <i>E21B 10/5673</i> (2013.01); <i>E21B 10/62</i> (2013.01); <i>E21B 10/633</i> (2013.01) | 9,623,542 B1     | 4/2017  | Miess et al.        |              |
| (58) | <b>Field of Classification Search</b> |                                                                                          | 9,714,545 B2     | 7/2017  | DiGiovanni et al.   |              |
|      | CPC .....                             | <i>E21B 10/5673</i> ; <i>E21B 2010/5673</i> ; <i>E21B 2010/562</i> ; <i>E21B 10/55</i>   | 9,732,563 B1     | 8/2017  | Mukhopadhyay        |              |
|      |                                       | See application file for complete search history.                                        | 9,650,839 B1     | 9/2017  | Miess               |              |
|      |                                       |                                                                                          | 9,759,015 B2     | 9/2017  | Miess               |              |
| (56) | <b>References Cited</b>               |                                                                                          | 9,844,854 B1     | 12/2017 | Gleason et al.      |              |
|      | U.S. PATENT DOCUMENTS                 |                                                                                          | D835,163 S       | 12/2018 | Mortensen et al.    |              |
|      | 3,894,673 A                           | 7/1975 Lowder et al.                                                                     | 2009/0260877 A1  | 10/2009 | Wirth               |              |
|      | 4,268,276 A                           | 5/1981 Bovenkerk                                                                         | 2010/0326740 A1  | 12/2010 | Hall et al.         |              |
|      | 4,274,900 A                           | 6/1981 Mueller et al.                                                                    | 2011/0031036 A1  | 2/2011  | Patel               |              |
|      | 4,410,054 A                           | 10/1983 Nagel et al.                                                                     | 2011/0147083 A1  | 6/2011  | Mauldin et al.      |              |
|      | 4,468,138 A                           | 8/1984 Nagel                                                                             | 2011/0171414 A1  | 7/2011  | Sreshtha et al.     |              |
|      | 4,560,014 A                           | 12/1985 Geczy                                                                            | 2012/0292188 A1  | 11/2012 | Kim et al.          |              |
|      | 4,592,682 A                           | 6/1986 Vanistendael                                                                      | 2012/0325563 A1  | 12/2012 | Scott et al.        |              |
|      | 4,629,373 A                           | 12/1986 Hall                                                                             | 2013/0068534 A1  | 3/2013  | DiGiovanni et al.   |              |
|      | 4,738,322 A                           | 4/1988 Hall et al.                                                                       | 2013/0068537 A1  | 3/2013  | DiGiovanni          |              |
|      | 4,811,801 A                           | 5/1989 Salesky et al.                                                                    | 2013/0263522 A1  | 10/2013 | Nilen et al.        |              |
|      | 4,893,859 A                           | 1/1990 Nash                                                                              | 2013/0292188 A1  | 11/2013 | Bilen et al.        |              |
|      | 4,913,247 A                           | 4/1990 Jones                                                                             | 2014/0318873 A1  | 10/2014 | Patel et al.        |              |
|      | 5,011,515 A                           | 4/1991 Frushour                                                                          | 2014/0367177 A1  | 12/2014 | Gonzalez et al.     |              |
|      | 5,016,718 A                           | 5/1991 Tandberg                                                                          | 2015/0266163 A1* | 9/2015  | Stockey .....       | B24D 18/0009 |
|      | 5,054,246 A                           | 10/1991 Phaal et al.                                                                     |                  |         |                     | 51/309       |
|      | D324,056 S                            | 2/1992 Frazee                                                                            | 2015/0292272 A1  | 10/2015 | Can et al.          |              |
|      | D324,226 S                            | 2/1992 Frazee                                                                            | 2015/0298292 A1  | 10/2015 | Can et al.          |              |
|      | 5,092,687 A                           | 3/1992 Hall                                                                              | 2018/0010396 A1  | 1/2018  | Dunbar et al.       |              |
|      | 5,120,327 A                           | 6/1992 Dennis                                                                            |                  |         |                     |              |
|      | 5,135,061 A                           | 8/1992 Newton, Jr.                                                                       |                  |         |                     |              |
|      | 5,154,245 A                           | 10/1992 Waldenstrom et al.                                                               |                  |         |                     |              |
|      | 5,172,778 A                           | 12/1992 Tibbitts et al.                                                                  |                  |         |                     |              |
|      | 5,364,192 A                           | 11/1994 Damm et al.                                                                      |                  |         |                     |              |
|      | 5,368,398 A                           | 11/1994 Damm et al.                                                                      |                  |         |                     |              |
|      | 5,460,233 A                           | 10/1995 Meany et al.                                                                     |                  |         |                     |              |
|      | 5,480,233 A                           | 1/1996 Cunningham                                                                        |                  |         |                     |              |
|      | 5,544,713 A                           | 8/1996 Dennis                                                                            |                  |         |                     |              |
|      | 5,601,477 A                           | 2/1997 Bunting et al.                                                                    |                  |         |                     |              |
|      | 5,662,720 A                           | 9/1997 O'Tighearnaigh                                                                    |                  |         |                     |              |
|      | 5,669,271 A                           | 9/1997 Griffin et al.                                                                    |                  |         |                     |              |
|      | 6,065,554 A                           | 5/2000 Taylor et al.                                                                     |                  |         |                     |              |
|      | 6,110,030 A                           | 8/2000 Hashimoto                                                                         |                  |         |                     |              |
|      | D436,820 S                            | 1/2001 Suzuki                                                                            |                  |         |                     |              |
|      | 6,302,410 B1                          | 10/2001 Wentworth et al.                                                                 |                  |         |                     |              |
|      | 6,338,754 B1                          | 1/2002 Cannon et al.                                                                     |                  |         |                     |              |
|      | 6,793,681 B1                          | 9/2004 Pope et al.                                                                       |                  |         |                     |              |
|      | D554,162 S                            | 10/2007 Hall et al.                                                                      |                  |         |                     |              |
|      | 7,464,973 B1                          | 12/2008 Chapman et al.                                                                   |                  |         |                     |              |
|      | D594,486 S                            | 7/2009 Morozov                                                                           |                  |         |                     |              |
|      | 7,845,438 B1                          | 12/2010 Vail et al.                                                                      |                  |         |                     |              |
|      | 7,866,418 B2                          | 1/2011 Bertagnolli et al.                                                                |                  |         |                     |              |
|      | 8,236,074 B1                          | 8/2012 Bertagnolli et al.                                                                |                  |         |                     |              |
|      | 8,261,858 B1                          | 9/2012 Atkins et al.                                                                     |                  |         |                     |              |
|      | 8,297,382 B2                          | 10/2012 Bertagnolli et al.                                                               |                  |         |                     |              |
|      | 8,596,387 B1                          | 12/2013 Sani et al.                                                                      |                  |         |                     |              |
|      | 8,734,552 B1                          | 5/2014 Vail et al.                                                                       |                  |         |                     |              |
|      | D708,238 S                            | 7/2014 Matti                                                                             |                  |         |                     |              |
|      | 8,807,247 B2                          | 8/2014 Scott et al.                                                                      |                  |         |                     |              |

## OTHER PUBLICATIONS

U.S. Appl. No. 12/961,787, filed Dec. 7, 2010, Mukhopadhyay et al.  
 U.S. Appl. No. 13/324,237, filed Dec. 13, 2011, Kidd et al.  
 U.S. Appl. No. 13/486,578, filed Jun. 1, 2012, Bertagnolli et al.  
 U.S. Appl. No. 13/734,354, filed Jan. 4, 2013, Linford et al.  
 U.S. Appl. No. 13/790,046, filed Mar 8, 2013, Cox.  
 U.S. Appl. No. 61/948,970, filed Mar. 6, 2014, Knuteson et al.  
 U.S. Appl. No. 14/273,360, filed May 8, 2014, Burton et al.  
 U.S. Appl. No. 14/275,574, filed May 12, 2014, Burton et al.  
 U.S. Appl. No. 62/002,001, filed May 22, 2014, Knuteson et al.  
 U.S. Appl. No. 14/627,966, filed Feb. 20, 2015, Linford et al.  
 U.S. Appl. No. 14/811,699, filed Jul. 28, 2015, Myers et al.  
 U.S. Appl. No. 62/232,732, filed Sep. 25, 2015, Weaver et al.  
 U.S. Appl. No. 62/279,271, filed Jan. 15, 2016, Mortensen et al.  
 U.S. Appl. No. 29/559,713, filed Mar. 30, 2016, Mortensen et al.  
 U.S. Appl. No. 61/891,525, filed Oct. 16, 2013, Miess.  
 U.S. Appl. No. 14/515,768, filed Oct. 16, 2014, Mortensen et al.  
 U.S. Appl. No. 14/515,768, Jan. 29, 2016, Restriction Requirement.  
 U.S. Appl. No. 14/515,768, May 31, 2016, Office Action.  
 U.S. Appl. No. 14/515,768, Nov. 14, 2016, Office Action.  
 U.S. Appl. No. 16/008,935, Jun. 14, 2018, Miess.  
 U.S. Appl. No. 14/515,768, Jul. 13, 2017, Office Action.  
 U.S. Appl. No. 14/515,768, Nov. 24, 2017, Notice of Allowance.  
 U.S. Appl. No. 14/515,768, Mar. 15, 2018, Notice of Allowance.  
 U.S. Appl. No. 29/559,713, Jan. 29, 2018, Restriction Requirement.  
 U.S. Appl. No. 14/515,768, Feb. 3, 2017, Advisory Action.  
 U.S. Appl. No. 14/515,768, Mar. 6, 2017, Non-Final Office Action.  
 U.S. Appl. No. 14/515,768, Jun. 27, 2018, Issue Notification.  
 U.S. Appl. No. 29/559,713, Jul. 19, 2018, Notice of Allowance.  
 U.S. Appl. No. 29/559,713, Nov. 14, 2018, Issue Notification.

\* cited by examiner



FIG. 1A



FIG. 1B



FIG. 2



FIG. 3



FIG. 4A



FIG. 4B



FIG. 4C



FIG. 5



FIG. 6



FIG. 7A



FIG. 7B



FIG. 7C



FIG. 7D



FIG. 8A



FIG. 8B



FIG. 8C



FIG. 8D



FIG. 8E



FIG. 8F



FIG. 8G



FIG. 8H

FIG. 8*i*







FIG. 10A



FIG. 10B



FIG. 10C



FIG. 10D



FIG. 10E



*FIG. 11*



*FIG. 12A*



FIG. 12B



FIG. 12C



*FIG. 12D*



*FIG. 12E*



*FIG. 12F*



*FIG. 12G*



FIG. 13



FIG. 14A



FIG. 14B

**POLYCRYSTALLINE DIAMOND  
COMPACTS, METHODS OF FABRICATING  
THE SAME, AND METHODS OF USING THE  
SAME**

**CROSS-REFERENCE TO RELATED  
APPLICATION(S)**

This application claims priority to U.S. Provisional Application No. 62/279,271 filed on 15 Jan. 2016, the disclosure of which is incorporated herein, in its entirety, by this reference.

**BACKGROUND**

Wear-resistant, polycrystalline diamond compacts (“PDCs”) are utilized in a variety of mechanical applications. For example, PDCs are used in drilling tools (e.g., cutting elements, gage trimmers, etc.), machining equipment, bearing apparatuses, wire-drawing machinery, and in other mechanical apparatuses.

PDCs have found particular utility as superabrasive cutting elements in rotary drill bits, such as roller-cone drill bits and fixed-cutter drill bits. A PDC cutting element typically includes a superabrasive diamond layer commonly known as a diamond table. The diamond table is formed and bonded to a substrate using a high-pressure/high-temperature (“HPHT”) process that sinters diamond particles under diamond-stable conditions. The PDC cutting element may also be brazed directly into a preformed pocket, socket, or other receptacle formed in a bit body. The substrate may optionally be brazed or otherwise joined to an attachment member, such as a cylindrical backing. A rotary drill bit typically includes a number of PDC cutting elements affixed to the bit body. It is also known that a stud carrying the PDC may be used as a PDC cutting element when attached to a bit body of a rotary drill bit by press-fitting, brazing, or otherwise securing the stud into a receptacle formed in the bit body.

Conventional PDCs are normally fabricated by placing a cemented carbide substrate into a container with a volume of diamond particles positioned on a surface of the cemented carbide substrate. A number of such containers may be loaded into an HPHT press. The substrate(s) and volume of diamond particles are then processed under HPHT conditions in the presence of a catalyst material that causes the diamond particles to bond to one another to form a matrix of bonded diamond grains defining a polycrystalline diamond (“PCD”) table. The catalyst material is often a metal-solvent catalyst (e.g., cobalt, nickel, iron, or alloys thereof) that is used for promoting intergrowth of the diamond particles.

In a conventional approach, a constituent of the cemented carbide substrate, such as cobalt from a cobalt-cemented tungsten carbide substrate, liquefies and sweeps from a region adjacent to the volume of diamond particles into interstitial regions between the diamond particles during the HPHT sintering process. The cobalt acts as a catalyst to promote intergrowth between the diamond particles, which results in formation of a matrix of bonded diamond grains having diamond-to-diamond bonding there between, with interstitial regions between the bonded diamond grains being occupied by the solvent catalyst.

The presence of the metal-solvent catalyst in the PCD table is believed to reduce the thermal stability of the PCD table at elevated temperatures. For example, the difference in thermal expansion coefficient between the diamond grains and the metal-solvent catalyst is believed to lead to chipping

or cracking of the PCD table during drilling or cutting operations, which can degrade the mechanical properties of the PCD table or cause failure. Additionally, some of the diamond grains can undergo a chemical breakdown or back-conversion to graphite via interaction with the solvent catalyst. At elevated high temperatures, portions of diamond grains may transform to carbon monoxide, carbon dioxide, graphite, or combinations thereof, thereby degrading the mechanical properties of the PDC.

One conventional approach for improving the thermal stability of a PDC is to at least partially remove the metal-solvent catalyst from the PCD table of the PDC by acid leaching. Another approach involves infiltrating and bonding an at least partially leached PCD table to a cemented carbide substrate with a metallic infiltrant, and acid leaching to at least partially remove the metallic infiltrant.

Despite the availability of a number of different PDCs, manufacturers and users of PDCs continue to seek PDCs that exhibit improved toughness, wear resistance, and thermal stability.

**SUMMARY**

PDCs, methods of fabricating the PDCs, and methods of using the PDCs are disclosed herein. The PDCs include a PCD table bonded to a substrate. The PCD table includes an upper surface having a plurality of recessed features formed therein. The plurality of recessed features function as stress concentrations that are configured to attract at least some cracks that form in the PCD table. As such, the plurality of recessed features limit or prevent propagation of the cracks into other portions of the PCD table and limit a volume of the PCD table that spalls during cutting operations. Methods of fabricating the PDCs include partially leaching the PCD table and, after leaching the PCD table, forming the plurality of recessed features in the upper surface thereof. Method of using the PDCs include rotating a PDC that has spalled relative to a rotary drill bit such that a portion of the upper surface of the PDC that has not spalled forms a cutting surface thereof. The disclosed PDCs may be used in a variety of applications, such as rotary drill bits, machining equipment, and other articles and apparatuses.

In an embodiment, a PDC is disclosed. The PDC includes a substrate. The PDC also includes a PCD table bonded to the substrate. The PCD table includes an interfacial surface bonded to the substrate, an upper surface spaced from the interfacial surface, and at least one lateral surface extending between the upper surface and the interfacial surface. The PCD table also includes a plurality of diamond grains bonded together defining a plurality of interstitial regions. The PCD table further includes an unleached region bonded to the interfacial surface. The unleached region includes at least one interstitial constituent disposed in at least a portion of the plurality of interstitial regions thereof. The PCD table also includes a leached region extending inwardly from the upper surface and at least a portion of the at least one lateral surface. The leached region is at least partially depleted of the at least one interstitial constituent. The PCD table additionally includes a plurality of recessed features extending from the upper surface through a portion of the polycrystalline diamond table. A majority of the plurality of recessed features do not extend into the unleached region.

In an embodiment, a method of fabricating a PDC is disclosed. The method includes leaching at least a portion of at least one interstitial constituent from a polycrystalline diamond table to a leach depth measured inwardly from an upper surface and at least one lateral surface of the poly-

crystalline diamond table to form a leached region. The method also includes, after leaching the polycrystalline diamond table, forming a plurality of recessed features that extend from the upper surface of the polycrystalline diamond table to a depth less than the leach depth of the leached region. Forming the plurality of recessed features forms a plurality of cells on the upper surface that are at least partially defined by the plurality of recessed features.

In an embodiment, a method of using a PDC is disclosed. The method includes decoupling at least one PDC from a drill bit body. The at least one PDC includes a PCD table bonded to a substrate. A portion of the PCD table includes a spalled region. The PCD table includes an interfacial surface bonded to the substrate, an upper surface spaced from the interfacial surface, and at least one lateral surface extending between the upper surface and the interfacial surface. The PCD table also includes a plurality of diamond grains bonded together defining a plurality of interstitial regions. The PCD table further includes a plurality of recessed features extending from the upper surface of the polycrystalline diamond table through a portion of the polycrystalline diamond table. At least one of the plurality of recessed features partially defines the spall region. Additionally, the PCD table includes an unleached region bonded to the interfacial surface. The unleached region includes an interstitial constituent disposed in at least a portion of the plurality of interstitial regions thereof. Finally, the PCD table includes a leached region extending inwardly from the upper surface and at least a portion of at least one lateral surface. The leached region is at least partially depleted of at least one interstitial constituent. A majority of the plurality of recessed features do not extend into the unleached region. The method also includes rotating the at least one PDC relative to the drill bit body to position a portion of the PCD table that does not include the spalled region in a cutting position. The method further includes coupling the at least one PDC to the drill bit body with the PCD table positioned in the cutting position.

In an embodiment, a PDC includes a substrate and a PCD table bonded to the substrate. The PCD table includes an interfacial surface bonded to the substrate, an upper surface spaced from the interfacial surface, and at least one lateral surface extending between the upper surface and the interfacial surface. The PCD table further includes a plurality of diamond grains bonded together defining a plurality of interstitial regions. The PCD table also includes an unleached region bonded to the interfacial surface, with the unleached region including at least one interstitial constituent disposed in at least a portion of the plurality of interstitial regions thereof; a leached region extending inwardly from the upper surface and at least a portion of the at least one lateral surface, with the leached region being at least partially depleted of the at least one interstitial constituent; and a plurality of recessed features extending from the upper surface through a portion of the PCD table, with the plurality of recessed features forming a plurality of cells. An initial spallation of the PCD table in response to a milling spallation test is about 10% or less of the area of the upper surface of the PCD table.

In an embodiment, a PDC includes a substrate and a PCD table bonded to the substrate. The PCD table includes an interfacial surface bonded to the substrate, an upper surface spaced from the interfacial surface, and at least one lateral surface extending between the upper surface and the interfacial surface. The PCD table further includes a plurality of diamond grains bonded together defining a plurality of interstitial regions. The PCD table also includes a plurality

of recessed features extending from the upper surface through a portion of the PCD table; an unleached region bonded to the interfacial surface, with the unleached region including at least one interstitial constituent disposed in at least a portion of the plurality of interstitial regions thereof; and a leached region extending inwardly from the upper surface and at least a portion of the at least one lateral surface, with the leached region being at least partially depleted of the at least one interstitial constituent. The PCD table exhibits a probability of failure less than about 0.4 at a distance cut of at least about 325 inches when tested in a milling spallation test.

Other embodiments include applications utilizing the disclosed PDCs in various articles and apparatuses, such as rotary drill bits, bearing apparatuses, wire-drawing dies, machining equipment, and other articles and apparatuses.

Features from any of the disclosed embodiments may be used in combination with one another, without limitation. In addition, other features and advantages of the present disclosure will become apparent to those of ordinary skill in the art through consideration of the following detailed description and the accompanying drawings.

#### BRIEF DESCRIPTION OF THE DRAWINGS

The drawings illustrate several embodiments of the present disclosure, wherein identical reference numerals refer to identical or similar elements or features in different views or embodiments shown in the drawings.

FIG. 1A is an isometric view of a PDC, according to an embodiment.

FIG. 1B is a side, cross-sectional view of the PDC shown in FIG. 1A taken along plane 1B-1B thereof.

FIG. 2 is a side, cross-sectional view of a PDC that includes a partially leached PCD table, according to an embodiment.

FIG. 3 is a schematic illustration of an embodiment of a method for fabricating a PDC that may be used in any of the embodiments disclosed herein, according to an embodiment.

FIGS. 4A-4C are partial, side, cross-sectional views of PCD tables that include at least one recessed feature formed therein that each exhibit different cross-sectional geometries, according to different embodiments.

FIGS. 5-10E are top plan views of PCD tables that exhibit different patterns of a plurality of recessed features formed in an upper surface thereof, according to different embodiments.

FIG. 11 is a photograph of a conventional PDC after the conventional PDC spalled.

FIGS. 12A-12G are photographs of different working examples of PDCs according to embodiments of the present disclosure, which include a plurality of recessed features formed thereon, after the different PDCs have spalled.

FIG. 13 is a graph showing probability of failure of comparative example 1 and working examples 2, 7, 8, and 9 versus distance each PDC cut prior to failure.

FIG. 14A is an isometric view of an embodiment of a rotary drill bit that may employ one or more of the disclosed PDC embodiments.

FIG. 14B is a top plan view of the rotary drill bit shown in FIG. 14A.

#### DETAILED DESCRIPTION

PDCs, methods of fabricating the PDCs, and methods of using the PDCs are disclosed herein. The PDCs include a PCD table bonded to a substrate. The PCD table includes an

upper surface having a plurality of recessed features formed therein. The plurality of recessed features function as stress concentrations that are configured to attract at least some cracks that form in the PCD table. As such, the plurality of recessed features limit or prevent propagation of the cracks into other portions of the PCD table and limit a volume or area of the PCD table that spalls during cutting operations. Methods of fabricating the PDCs include partially leaching the PCD table and, after leaching the PCD table, forming the plurality of recessed features in the upper surface thereof. Method of using the PDCs include rotating a PDC that has spalled relative to a rotary drill bit such that a portion of the upper surface of the PDC that has not spalled forms a cutting surface thereof. The disclosed PDCs may be used in a variety of applications, such as rotary drill bits, machining equipment, and other articles and apparatuses.

FIG. 1A is an isometric view of a PDC 100, according to an embodiment. The PDC 100 includes a PCD table 102 bonded to a substrate 104. The PCD table 102 includes an upper surface 106 that forms at least part of a working surface of the PDC 100. The upper surface 106 includes a plurality of recessed features 108 (e.g., grooves) formed therein. In an embodiment, during cutting operations using the PDC 100, cracks may form in the PCD table 102. The plurality of recessed features 108 function as stress concentrations that are configured to attract cracks thereto, thereby limiting crack propagation into the PCD table 102 during cutting operations. As such, the plurality of recessed features 108 may limit spalling to a limited region of the PCD table 102 ("spalled region"). Additionally, the plurality of recessed features 108 limit crack propagation from the spalled region to other regions of the PCD table 102. In an embodiment, the plurality of recessed features 108 may be sized and configured to limit a spalled region to 10% or less, 5% of less, 4% or less, or 3% or less, about 3% to about 10%, about 5% to about 8%, or about 4% to about 7% of a total surface area of the upper surface 106. As such, the plurality of recessed features 108 may help maintain one or more of a structural integrity, a strength, or a toughness of the PCD table 102.

In some embodiments, a probability of failure as determined in a milling spallation test, which is described in comparative example 1 below, may be less than about 0.1 at a distance cut of about 315 inches or greater (e.g., about 315 inches to about 325 inches, about 325 inches to about 350, about 350 inches or greater), may be less than about 0.3 to about 0.4 at a distance cut of about 325 inches or greater (e.g., about 325 inches to about 350 inches, about 350 inches to about 375 inches, at least about 350 inches, at least about 375 inches, about 375 inches to about 400 inches, or greater than 400 inches), may be less than about 0.75 at a distance cut of about 340 inches or greater (e.g., about 350 inches to about 375 inches, about 375 inches to about 400 inches, about 400 inches to about 425 inches, about 425 inches or greater).

The substrate 104 may include a cemented carbide material. For example, the substrate 104 may include tungsten carbide, titanium carbide, chromium carbide, niobium carbide, tantalum carbide, vanadium carbide, or combinations thereof that may be cemented with iron, nickel, cobalt, combinations thereof, or alloys thereof. For example, the substrate 104 may comprise a cobalt-cemented tungsten carbide. In some embodiments, the substrate 104 may be omitted (e.g., a free-standing PCD table).

The PCD table 102 includes an interfacial surface 110 that is spaced from the upper surface 106 and bonded to the substrate 104. The interfacial surface 110 may be substan-

tially planar (FIG. 1B), exhibit a concave or convex curvature, or have one or more recesses and/or protrusions formed therein. The substrate 104 may include a surface that substantially corresponds to the interfacial surface 110. The PCD table 102 may also include at least one lateral surface 112 that extends from the interfacial surface 110 to the upper surface 106. In some embodiments, the PCD table 102 may include an optional chamfer 114 extending between the at least one lateral surface 112 and the upper surface 106. In other embodiments, the PCD table 102 may include a rounded edge, multiple chamfers (e.g., double chamfer), or any other suitable edge geometry.

In the illustrated embodiments shown in FIGS. 1A-1B, the PDCs are cylindrical. However, in other embodiments, the PDCs disclosed herein may exhibit other suitable configurations (e.g., triangular, rectangular, elliptical, or other suitable configuration) that may exhibit one or more peripheral surfaces or sides.

The PCD table 102 includes a plurality of directly bonded together diamond grains that exhibit diamond-to-diamond bonding therebetween (e.g.,  $sp^3$  bonding). The plurality of directly bonded together diamond grains define a plurality of interstitial regions therebetween. The PCD table 102 may include at least one interstitial constituent that at least partially occupies at least some of the interstitial regions of the PCD table 102. The at least one interstitial constituent may include at least one of a metal-solvent catalyst (e.g., cobalt, iron, nickel, combinations thereof, or alloys thereof), at least one constituent from the substrate (e.g., tungsten and/or tungsten carbide), a nonmetallic catalyst (e.g., one or more alkali metal carbonates, one or more alkaline metal carbonates, one or more alkaline earth metal hydroxides, or combinations thereof), or another suitable interstitial constituent.

The at least one interstitial constituent may be at least partially leached from the PCD table 102. For example, FIG. 1B is a side, cross-sectional view of the PDC 100 shown in FIG. 1A taken along plane 1B-1B thereof. The PCD table 102 includes an unleached region 116 that is bonded to the substrate 104. The unleached region 116 may extend from the interfacial surface 110 towards the upper surface 106. The unleached region 116 is a portion of the PCD table 102 that is not leached and includes the at least one interstitial constituent therein that at least partially occupies (e.g., at least substantially occupies) at least some of the interstitial regions thereof.

The PCD table 102 also includes a leached region 118 that extends inwardly from the upper surface 106, at least a portion of the at least one lateral surface 112, and the optional chamfer 114. For example, an interface 119 is located between the leached region 118 and the unleached region 116. The leached region 118 includes at least some of the at least one interstitial constituent removed from the interstitial regions thereof (e.g., the leached region 118 exhibits a lower concentration of the at least one interstitial constituent than the unleached region 116). For example, a residual amount of the at least one interstitial constituent may still remain in the interstitial regions of the leached region 118 after leaching. The residual amount of the at least one interstitial constituent in the interstitial regions of the leached region 118 may be about 0.5% to about 2% by weight (e.g., about 0.8% to about 1.2% by weight), or less than about 0.5% by weight (e.g., substantially completely removed from the interstitial regions of the leached region 118). In an embodiment, the leached region 118 may extend inwardly along at least about 50% of a length of the at least one lateral surface 112 (i.e., from the interfacial surface 110

to a bottommost edge 123 of the chamfer 114), such as along at least about 75% of the at least one lateral surface 112, along at least about 80% of the at least one lateral surface 112, or along at least about 90% of the at least one lateral surface 112. As will be discussed later, increasing the percentage of the at least one lateral surface 112 that is leached may allow the  $L_1^*$  value to increase (FIG. 2).

The leached region 118 may exhibit a first leach depth  $D_1$  measured substantially perpendicularly inwardly from the upper surface 106 to the interface 119 between the leached region 118 and the unleached region 116. The first leach depth  $D_1$  may be about 200  $\mu\text{m}$  to about 900  $\mu\text{m}$ . For example, the first leach depth  $D_1$  may be about 200  $\mu\text{m}$  to about 400  $\mu\text{m}$ , about 400  $\mu\text{m}$  to about 500  $\mu\text{m}$ , about 500  $\mu\text{m}$  to about 800  $\mu\text{m}$ , about 800  $\mu\text{m}$  to about 900  $\mu\text{m}$ , less than 200  $\mu\text{m}$ , or greater than 900  $\mu\text{m}$ . In an embodiment, the first leach depth  $D_1$  may be substantially uniform along a selected length of the upper surface 106. In an embodiment, the first leach depth  $D_1$  may vary along a selected length of the upper surface 106. For example, as will be discussed in more detail below, the first leach depth  $D_1$  may be greater at and/or near an edge of the upper surface 106 (e.g., where the upper surface 106 meets the at least one lateral surface 112, the chamfer 114, etc.) than a location spaced from the edge of the upper surface 106. The leached region 118 may also exhibit leach depths measured substantially perpendicularly inwardly from the chamfer 114 and the at least one lateral surface 112, respectively. In an embodiment, the leach depth measured substantially perpendicularly inwardly from at least a portion of the chamfer 114 and at least a portion of the at least one lateral surface 112 may be substantially the same as or similar to the first leach depth  $D_1$ . In another embodiment, the leached depth measured substantially perpendicularly inwardly from at least a portion of the chamfer 114 and/or a portion of the at least one lateral surface 112 may be different than the first leach depth  $D_1$ . For example, the leach depth measured substantially perpendicularly inwardly from a portion of the at least one lateral surface 112 may be greater than the first leach depth  $D_1$ . Additional examples of leach profiles that the leached region 118 may exhibit are disclosed in U.S. Pat. No. 8,596,387, the disclosure of which is incorporated herein, in its entirety, by this reference.

The leach profile (e.g., the leach depth measured inwardly from the upper surface 106, the at least one lateral surface 112, and/or the optional chamfer 114) may be used to predict when the PDC 100 spalls. FIG. 1B illustrates a predicted initial wear front 120 before the PDC 100 has been used and experienced wear. The predicted initial wear front 120, in an embodiment, may be represented as an idealized, hypothetical plane that extends at an angle  $\theta$  relative to the at least one lateral surface 112. The angle  $\theta$  may be about 10° to about 30°, such as about 20°. The predicted initial wear front 120 also exhibits a single point of tangency with a portion of the PCD table 102. For example, in the illustrated embodiment, the predicted initial wear front 120 may intersect (e.g., at a single point) with a bottommost edge 123 of the chamfer 114. In another example, the predicted initial wear front 120 may intersect (e.g., at a single point) an outer edge of the upper surface 106, one or more portions of the upper surface 106 (e.g., the upper surface 106 exhibits a convex curvature), or any other portion or portions of the PDC 100.

During operation, portions of the PCD table 102 may generally wear away along an expected wear front 122. In an embodiment, the expected wear front 122 may be assumed to be generally parallel to the predicted initial wear front 120. In such an embodiment, the expected wear front 122

may be a plane that extends at the angle  $\theta$  relative to the at least one lateral surface 112. The inventors currently believe that at least one or more microscopic cracks or other defect forms near the interface 119 between the leached region 118 and the unleached region 116 when the expected wear front 122 extends through the leached region 118 and contacts the unleached region 116. The inventors currently believe that the cracks and/or other defect(s) may form a leach boundary-wear intersection location 124 that increases a likelihood that the PCD table 102 spalls.

The PCD table 102 may be expected to spall in response to the expected wear front 122 intersecting with the interface 119 between the unleached region 116 and the leached region 118 (e.g., the first location where the leach boundary-wear intersection location 124 may form). The shortest distance measured substantially perpendicularly from the predicted initial wear front 120 (e.g., having an angle  $\theta$  of about 20°) and the interface 119 is referred to as the  $L_1^*$  value (e.g., the distance measured substantially perpendicularly between the predicted initial wear front 120 and the subsequent expected wear front 122 intersecting with the interface 119). In other words, the  $L_1^*$  value is the expected amount of wear into the PCD table 102 before the PCD table 102 becomes more susceptible to spallation. In the illustrated embodiment, the  $L_1^*$  value is measured between the predicted initial wear front 120 and a portion of the interface 119 that is spaced from the at least one lateral surface 112.

The leach profile of the leached region 118 may be configured to maximize the  $L_1^*$  value. For example, in the illustrated embodiment, increasing one or more of the first leach depth  $D_1$ , the leach depth measured inwardly from the chamfer 114, or the leach depth measured inwardly from the at least one lateral surface may increase the  $L_1^*$  value. In particular, increasing the leach depth measured inwardly from the at least one lateral surface may increase the  $L_1^*$  value more than increasing the first leach depth  $D_1$ . Additionally, forming the chamfer 114 in the PCD table 102 prior to leaching the PCD table 102 may also increase the  $L_1^*$  value. In an embodiment, the  $L_1^*$  value may be about 50  $\mu\text{m}$  to about 1200  $\mu\text{m}$ . For example, the  $L_1^*$  value may be about 100  $\mu\text{m}$  to about 600  $\mu\text{m}$ , about 100  $\mu\text{m}$  to about 250  $\mu\text{m}$ , about 250  $\mu\text{m}$  to about 500  $\mu\text{m}$ , 500  $\mu\text{m}$  to about 750  $\mu\text{m}$ , or about 750  $\mu\text{m}$  to about 1000  $\mu\text{m}$ . In an embodiment, the  $L_1^*$  value may be less than 50  $\mu\text{m}$  or greater than 1200  $\mu\text{m}$ .

As previously discussed, the PCD table 102 includes the plurality of recessed features 108 formed in the upper surface 106. At least a portion of the plurality of recessed features 108 may also be formed in the at least one lateral surface 112 and/or the chamfer 114. The plurality of recessed features 108 are configured to limit crack propagation and/or spallation in the PCD table 102. In particular, a crack in the PCD table 102 (e.g., formed at the leach boundary-wear intersection location 124) may be attracted to the nearest recessed feature 108 because the nearest recessed feature 108 serves as a stress concentration and a path of least resistance for crack propagation thereto. As such, the plurality of recessed features 108 may limit crack propagation into other regions of the PCD table 102, thereby maintaining a strength and/or a toughness of the other regions of the PCD table 102. For example, a crack may cause a portion of the PCD table 102 to spall. However, since the crack may be attracted to nearby recessed feature 108, the plurality of recessed features 108 may limit the amount of the PCD table 102 that spalls. For instance, at least a portion at least one of the plurality of recessed features 108 may at least partially define a spalled region or area formed in the PCD table 102. The spalled region may

be less than 10% the total area of the upper surface **106**, such as less than 5%, less than 4%, less than 3%, less than 2%, less than 1%, or less than 5% of a total surface area of the upper surface **106**.

Each of the plurality of recessed features **108** includes a base **126** that partially defines each recessed feature **108**. The base **126** is the portion of each of the plurality of recessed features **108** that is farthest spaced from the upper surface **106**. A depth  $D_3$  of each of the plurality of recessed features **108** is measured substantially perpendicularly from the upper surface **106** (e.g., an imaginary continuation of the upper surface **106** that extends over the recessed feature **108**) to the base **126**. In an embodiment, the depth  $D_3$  of each of the plurality of recessed features **108** may be about 50  $\mu\text{m}$  to about 500  $\mu\text{m}$ , such as about 50  $\mu\text{m}$  to about 150  $\mu\text{m}$ , 100  $\mu\text{m}$  to about 250  $\mu\text{m}$ , 200  $\mu\text{m}$  to about 400  $\mu\text{m}$ , or about 300  $\mu\text{m}$  to about 500  $\mu\text{m}$ . In an embodiment, the depth  $D_3$  of each of the plurality of recessed features **108** may be less than about 50  $\mu\text{m}$  or greater than 500  $\mu\text{m}$ . The depth  $D_3$  of each of the plurality of recessed features **108** may be selected based on a width or area of the respective recessed feature **108**, the cross-sectional shape (in side view) of the respective recessed feature **108**, the first leach depth  $D_1$ , the  $L_1^*$  value, the shortest distance between the leach boundary-wear intersection location **124** and the respective recessed feature **108**, the application of the PDC **100**, etc.

In an embodiment, the plurality of recessed features **108** may potentially adversely affect the strength and toughness of the PCD table **102**. For example, the strength and/or toughness of the PCD table **102** may decrease as an average depth of the plurality of recessed features **108** increases. However, the ability of the plurality of recessed features **108** to attract cracks thereto may also increase as the average depth of the plurality of recessed features **108** increases. For example, a recessed feature **108** that is positioned proximate to the leach boundary-wear intersection location **124** or that exhibits a relatively high stress concentration factor may exhibit a depth that is relatively shallow (e.g., about 50  $\mu\text{m}$  to about 250  $\mu\text{m}$ ). In another embodiment, a recessed feature **108** that is spaced from leach boundary-wear intersection location **124** or that exhibits a relatively low stress concentration factor may exhibit a depth that is relatively deep (e.g., about 250  $\mu\text{m}$  to about 500  $\mu\text{m}$ , greater than 500  $\mu\text{m}$ ).

In an embodiment, at least some of the plurality of recessed features **108** only extend partially through or within the leached region **118**. As such, the leach depth of the remaining leached region **118** proximate to the at least some of the plurality of recessed features **108** may be decreased. For example, the leached region **118** may exhibit a second leach depth  $D_2$  measured substantially perpendicularly inwardly from the base **126** of each of the at least some of the plurality of recessed features **108** to the interface **119** between the leached region **118** and the unleached region **116**. In an embodiment, the second leach depth  $D_2$  may be about 1% to about 75% less than the first leach depth  $D_1$ . For example, the second leach depth  $D_2$  may be about 1% less than to about 5% less than, about 5% less than to about 25% less than, about 20% less than to about 40% less than, about 25% less than to about 50% less than, or about 50% less than to about 75% less than the first leach depth  $D_1$ . For example, if  $D_1$  equals about 500  $\mu\text{m}$ , then  $D_2$  may be about 20% less than to about 40% less than  $D_1$  (i.e., 300  $\mu\text{m}$  to about 400  $\mu\text{m}$ ). In another embodiment, the second leach depth  $D_2$  may be greater than 0% to about 1% less than the first leach depth  $D_1$ , about 75% less than the first leach depth  $D_1$  to completely through the leached region **118**, or about 75% less than the first leach depth  $D_1$  to substantially through the PCD

table **102**. As previously discussed, the percentage of the second leach depth  $D_2$  to the first leach depth  $D_1$  may potentially affect the performance of the PDC **100**. For example, the second leach depth  $D_2$  of at least some of the plurality of recessed features **108** may be significantly less than the first leach depth  $D_1$  (e.g., about 50% to about 75% less than the first leach depth  $D_1$ ) when the recessed features **108** are positioned proximate to the anticipated leach boundary-wear intersection location **124** and/or exhibits a relatively high stress concentration factor.

In an embodiment, the first leach depth  $D_1$  may be about 1.33 to about 20 times greater than the depth  $D_3$  of at least some of the plurality of recessed features **108**. For example, the first leach depth  $D_1$  may be about 1.5 to about 5, about 2 to about 10, about 5 to about 15, about 10 to about 15, or about 15 to about 20 times greater than the depth  $D_3$  of at least some of the plurality of recessed features **108**. In an embodiment, the first leach depth  $D_1$  may be about 1.0 to about 1.33 times greater or more than 20 times greater than depth  $D_3$  of at least some of the plurality of recessed features **108**. In an embodiment, the depth  $D_3$  of at least some of the plurality of recessed features **108** may be greater than the first leach depth  $D_1$ . As previously discussed, the depth  $D_3$  of the plurality of recessed features **108** relative to the first leach depth  $D_1$  may affect to the performance of the PDC **100**. For example, the first leach depth  $D_1$  may be at least about 4 times greater than the depth  $D_3$  of at least some of the plurality of recessed features **108** when the recessed features **108** are positioned proximate to the anticipated leach boundary-wear intersection location **124** and/or exhibits a relatively high stress concentration factor.

In an embodiment, the depth  $D_3$  of at least some of the plurality of recessed features **108** may vary with location along the upper surface **106**. For example, the depth of at least some of the plurality of recessed features **108** may generally increase, decrease, undulate, or vary from a location on the upper surface **106** (e.g., a center of the upper surface **106**) towards an edge of the upper surface **106**. For example, the depth  $D_3$  of at least some of the plurality of recessed features **108** may be greatest at and/or near the edge of the upper surface **106**. As another example, the depth  $D_3$  of at least some of the plurality of recessed features **108** may be smallest at and/or near the edge of the upper surface **106**. In an embodiment, the depth  $D_3$  of at least some of the plurality of recessed features **108** may be greatest at, near, and/or inwardly from a location where the expected wear front **122** contacts the unleached portion **116**. Varying the depth  $D_3$  of at least some of the plurality of recessed features **108** may increase the overall strength and toughness of the PCD table **102** because the average depth of the plurality of recessed features **108** is less than the greatest depth of the plurality of recessed features **108**. However, the depth of the plurality of recessed features **108** may be sufficiently deep at certain locations to limit a spalled region formed in the PCD table **102**.

In an embodiment, the plurality of recessed features **108** may be formed in only a selected portion of the upper surface **106**. Forming the plurality of recessed features **108** in a selected portion of the upper surface **106** may increase the strength and toughness the PCD table **102**. For example, the plurality of recessed features **108** may be formed in a radially outer half of the upper surface **106**. The plurality of recessed features **108** may be formed in the radially outer half of the upper surface **106** because the leach boundary-wear intersection location **124** may be more likely to occur in the radially outer half of the PCD table **102**. In an embodiment, the plurality of recessed features **108** may be

## 11

formed over the entire upper surface **106** (e.g., uniformly formed on the upper surface **106**). For example, forming recessed features **108** in the radially inner half of the upper surface **106** may act as a redundant spallation limiting structure for the plurality of recessed features **108** formed in the radially outer half of the upper surface **106**.

In an embodiment, at least some of the plurality of recessed features **108** may extend to an outer edge of the upper surface **106**. However, at least some of the plurality of recessed features **108** may extend to other portions of the PCD table **102**. For example, at least some of the plurality of recessed features **108** may extend from a location on the upper surface **106** to a location inwardly from outer edge of the upper surface **106**. In another example, at least some of the plurality of recessed features **108** may extend from a location on the upper surface **106** to a location beyond the outer edge of the upper surface **106**, such as to a location on the chamfer **114** or a location on the at least one lateral surface **112**.

The ability of the plurality of recessed features **108** to attract cracks and/or limits spallation may be dependent on the plurality of recessed features' **108** stress concentration factor. In an embodiment, the stress concentration factor of the plurality of recessed features **108** may increase as a ratio of the average depth of the plurality of recessed features **108** to an average width of the plurality of recessed features **108** increases. For example, the ratio may be at least about 1, at least about 1.5, at least about 2, at least about 3, or about 1.5 to about 3.

The plurality of recessed features **108** may exhibit a spacing therebetween configured to cause cracks formed at or near the leach boundary-wear intersection location **124** to be attracted to the nearest recessed feature **108**. In an embodiment, two substantially similar immediately adjacent recessed features may be substantially parallel along a selected length thereof. The distance between the substantially parallel lengths of the two immediately adjacent recessed features may be less than about 3 mm, such as less than about 2 mm, less than about 1 mm, about 1 mm to about 3 mm, or about 0.5 mm to about 2 mm. The inventors have found that the two recessed features can exhibit a microscopic spacing therebetween and a propagating crack is still attracted to the nearest recessed feature. In particular, the inventors have found that the two recessed features may exhibit a spacing therebetween of about 650  $\mu\text{m}$  or less (e.g., about 625  $\mu\text{m}$  or less, about 600  $\mu\text{m}$  or less, about 500  $\mu\text{m}$  or less, about 400  $\mu\text{m}$  or less, about 300  $\mu\text{m}$  or less, or about 250  $\mu\text{m}$  or less, about 250  $\mu\text{m}$  to about 500  $\mu\text{m}$ , or about 300  $\mu\text{m}$  to about 500  $\mu\text{m}$ ) and the propagating crack can still be attracted to the nearest recessed feature.

Referring to FIG. 1A, the upper surface **106** may include a plurality of cells **128** (e.g., closed cells or partially closed cells) formed therein. The plurality of cells **128** may be at least partially defined by the plurality of recessed features **108**. At least some of the plurality of cells **128** may also be partially defined by at least one of the at least one lateral surface **112** and/or the optional chamfer **114**. Each of the plurality of cells **128** may define a portion of the upper surface **106** that may break from the upper surface **106** when the PCD table **102** spills. As such, each of the plurality of cells **128** may be configured to limit a volume or area of the upper surface **106** that breaks from the upper surface **106**. For example, the plurality of cells **128** may exhibit an average surface area that is less than about 5% of the surface area of the upper surface **106**. For example, the plurality of cells **128** may exhibit an average surface area that is less than about 4%, less than about 3%, less than about 2%, less

## 12

than about 1%, or about 1% to about 5% of the surface area of the upper surface **106**. For example, the plurality of cells may exhibit an average surface area that is greater than about 20  $\text{mm}^2$ , about 0.25  $\text{mm}^2$  to about 20  $\text{mm}^2$ , about 10  $\text{mm}^2$  to about 15  $\text{mm}^2$ , about 5  $\text{mm}^2$  to about 10  $\text{mm}^2$ , about 1  $\text{mm}^2$  to about 5  $\text{mm}^2$ , about 2  $\text{mm}^2$  to about 4  $\text{mm}^2$ , or about 0.5  $\text{mm}^2$  to about 3  $\text{mm}^2$ . As such, when one or more of the plurality of cells **128** break from the upper surface **106**, the percentage of the total surface area of the upper surface **106** (prior to any wear, damage, or spallation) that breaks away is less than about 5%, less than about 7.5%, less than about 10%, less than about 12.5%, less than about 15%, less than about 20%, less than about 25%, about 5% to about 15%, about 5% to about 10%, about 10% to about 20%, or about 15% to about 25%. In a specific example, if the total surface area of the upper surface **106** equals about 201  $\text{mm}^2$ , then less than about 5% would be about 10  $\text{mm}^2$  or less.

FIG. 2 is a side, cross-sectional view of a PDC **200** that includes a partially leached PCD table **202**, according to an embodiment. Except as otherwise disclosed herein, the PDC **200** may be substantially the same as or similar to the PDC **100** shown in FIGS. 1A-1B. For example, the PCD table **202** includes an unleached region **216** that is bonded to a substrate **104**, a leached region **218**, and an interface **219** therebetween. The leached region **218** extends inwardly from an upper surface **206**, at least one lateral surface **212**, and optionally a chamfer **214** of the PCD table **202**.

FIG. 2 illustrates a predicted initial wear front **220** prior to the PDC **200** being worn. The predicted initial wear front **220** is shown as a surface that extends at an angle  $\theta$  relative to the at least one lateral surface **212**. The angle  $\theta$  may be about 10° to about 30°, such as about 20°. The predicted initial wear front **220** may intersect the PCD table **202** (e.g., at a bottommost portion of the chamfer **214**). During operation, the PCD table **202** may generally wear along an expected wear front **222** that is substantially congruent to the predicted initial wear front **220**. Similar to the PCD table **102** (FIG. 1B), a leach boundary-wear intersection location **224** may form when the expected wear front **222** first contacts the unleached region **216**. The PCD table **202** may exhibit an  $L_1^*$  value, which is the distance between the predicted initial wear front **220** and the expected wear front **222** when the expected wear front **222** contacts the unleached region **216** (e.g., when the angle  $\theta$  is about 20°, the shortest distance measured substantially perpendicularly from the predicted initial wear front **220** to a portion of the interface **219**). In the illustrated embodiment, the expected wear front **222** contacts the unleached region **216** (where the interface **219** contacts the at least one lateral surface **212**). As such, unlike the PCD table **102** (FIG. 1B), increasing the first leach depth  $D_1$ , the leach depth measured inwardly from the at least one lateral surface **212** and/or the leach depth measured inwardly from the optional chamfer **214** does not increase the  $L_1^*$  value. Instead, the  $L_1^*$  value only increases when the percentage of the at least one lateral surface **212** is leached. Therefore, in some embodiments, the  $L_1^*$  value illustrated in FIG. 2 may be the maximum possible  $L_1^*$  value.

The PCD table **202** may include a plurality of recessed features **208** formed in the upper surface **206**. In the illustrated embodiment, the leach boundary-wear intersection location **224** may be spaced relatively far from the upper surface **206**. As such, in an embodiment, the plurality of recessed features **208** may exhibit a relatively great depth (e.g., 500  $\mu\text{m}$  or greater), an average depth that is greater than an average width thereof (e.g., by a ratio of about 2 or

more), and/or another feature configured to attract cracks to the nearest recessed feature **208** and/or limit spallation.

FIG. 3 is a schematic illustration of an embodiment of a method for fabricating a PDC **300** that may be used in any of the embodiments disclosed herein, according to an embodiment. Referring to FIG. 3, a mass of diamond particles **330** is positioned adjacent to a substrate **104**. The mass of diamond particles **330** may exhibit an average particle size of about 0.1  $\mu\text{m}$  to about 150  $\mu\text{m}$  (e.g., about 50  $\mu\text{m}$  or less, about 30  $\mu\text{m}$  or less, about 20  $\mu\text{m}$  or less, about 20  $\mu\text{m}$  to about 18  $\mu\text{m}$ , or about 15  $\mu\text{m}$  to about 18  $\mu\text{m}$ ). The diamond particle size distribution of the mass of diamond particles **330** may exhibit a single mode, or may exhibit a bimodal or greater grain size distribution. In an embodiment, the plurality of diamond particles may include a relatively larger size and at least one relatively smaller size. As used herein, the phrases “relatively larger” and “relatively smaller” refer to particles sizes determined by any suitable method, which differ by at least a factor of two (e.g., 40  $\mu\text{m}$  and 20  $\mu\text{m}$ ). In various embodiments, the diamond particles **330** may include a portion exhibiting a relatively larger size (e.g., 100  $\mu\text{m}$ , 90  $\mu\text{m}$ , 80  $\mu\text{m}$ , 70  $\mu\text{m}$ , 60  $\mu\text{m}$ , 50  $\mu\text{m}$ , 40  $\mu\text{m}$ , 30  $\mu\text{m}$ , 20  $\mu\text{m}$ , 15  $\mu\text{m}$ , 12  $\mu\text{m}$ , 10  $\mu\text{m}$ , 8  $\mu\text{m}$ ) and another portion exhibiting at least one relatively smaller size (e.g., 30  $\mu\text{m}$ , 20  $\mu\text{m}$ , 10  $\mu\text{m}$ , 15  $\mu\text{m}$ , 12  $\mu\text{m}$ , 10  $\mu\text{m}$ , 8  $\mu\text{m}$ , 4  $\mu\text{m}$ , 2  $\mu\text{m}$ , 1  $\mu\text{m}$ , 0.5  $\mu\text{m}$ , less than 0.5  $\mu\text{m}$ , 0.1  $\mu\text{m}$ , less than 0.1  $\mu\text{m}$ ). Of course, the diamond particles **330** may also include three or more different sizes (e.g., one relatively larger size and two or more relatively smaller sizes), without limitation. Examples of diamond particle size distributions for the diamond particles **300** are disclosed in U.S. Provisional Patent Application No. 61/948,970, U.S. Provisional Patent Application No. 62/002,001, U.S. patent application Ser. No. 13/734,354, and U.S. patent application Ser. No. 14/627,966. The disclosure of each of the foregoing patent applications is incorporated herein, in its entirety, by this reference.

In order to effectively HPHT sinter the mass of diamond particles **330**, the mass of diamond particles **330** may be placed adjacent a surface of the substrate **104** to form an assembly **332**. The assembly **332** may be placed in a pressure transmitting medium, such as a refractory metal can, graphite structure, pyrophyllite, combinations thereof, or another suitable container or supporting element. The pressure transmitting medium, including the assembly **332**, may be subjected to an HPHT process at a temperature of at least about 1000° C. (e.g., about 1100° C. to about 2200° C., or about 1200° C. to about 1450° C.) and a pressure in the pressure transmitting medium of at least about 5 GPa (e.g., at least about 7.5 GPa, at least about 9.0 GPa, at least about 10.0 GPa, at least about 11.0 GPa, at least about 12.0 GPa, at least about 14.0, or about 7.5 GPa to about 9.0 GPa) for a time sufficient to sinter the diamond particles **330** and form a PCD table **302** bonded to the substrate **104** thereby forming the PDC **300**.

During the HPHT process, the presence of a catalyst facilitates intergrowth between the mass of diamond particles **330** and forms the PCD table **302** including directly bonded-together diamond grains (e.g., exhibiting  $\text{sp}^3$  bonding) defining a plurality of interstitial regions. In the illustrated embodiment, the PDC **300** may be formed by sintering the mass of diamond particles **330** on the substrate **104**, which may be a cobalt-cemented tungsten carbide substrate. For example, cobalt and/or a cobalt alloy from the substrate **104** liquefies during the HPHT process and infiltrates into the mass of diamond particles **330** to catalyze formation of the PCD table **302**. In such an example, some tungsten

and/or tungsten carbide (metallic infiltrants) from the substrate **104** may dissolve in or otherwise transfer or alloy with the catalyst. However, in other embodiments, the catalyst may be mixed with the mass of diamond particles **330**, provided from a thin foil, another external source, or combinations thereof. Additionally, the catalyst and the metallic infiltrants may react with the mass of diamond particles **330** to form carbides. As such, the interstitial regions of the PCD table **302** may be at least partially occupied by at least one interstitial constituent (e.g., at least one of a metal-solvent catalyst, a metallic infiltrant, one or more formed carbides etc.).

The PCD table **302** so formed may include an interfacial surface **310** bonded to the substrate **104**. Examples of interfacial surface geometries for the substrate **104** that may be bonded to the interfacial surface **310** are disclosed in U.S. Pat. No. 8,297,382, the disclosure of which is incorporated herein, in its entirety, by this reference. The PCD table **302** may include an upper surface **306** spaced from the interfacial surface **310** and at least one lateral surface **312** extending between the upper surface **306** and the interfacial surface **310**. In an embodiment, the sintered grains of the PCD table **302** may exhibit an average grain size of about 20  $\mu\text{m}$  or less or about 30  $\mu\text{m}$  or less. For example, the average grain size and grain size distribution of the PCD table **302** may be substantially similar or the same as the average diamond particle size and distribution of the mass of diamond particles **330**.

Examples of suitable HPHT process conditions that may be used to form any of the PDC embodiments disclosed herein are disclosed in U.S. Pat. No. 7,866,418 which is incorporated herein, in its entirety, by this reference.

After the HPHT process, the PDC **300** may be subsequently shaped to include an optional peripherally-extending chamfer **314**. Further, as previously described, the PCD table **302** may be at least partially leached to remove at least a portion of the at least one interstitial constituent therefrom. In an embodiment, the PDC **300** may be at least partially immersed in and/or exposed to a leaching agent (e.g., hydrofluoric acid, nitric acid, a supercritical fluid, a gaseous leaching agent, another suitable leaching agent, or combinations thereof) to at least partially remove at least one interstitial constituent from the PCD table **302** to form a leached region (e.g., leach regions **118**, **218** of FIGS. 1B-2). Removing at least a portion of the at least one interstitial constituent from the PCD table **302** may improve the wear resistance, heat resistance, thermal stability, or combinations thereof of the PCD table **302**, particularly in situations where the PCD table **302** may be exposed to elevated temperatures.

In an embodiment, the PCD table **302** may include a plurality of recessed features **308** formed in the upper surface **306** thereof after the PCD table **302** is at least partially leached. For example, the plurality of recessed features **308** may be formed in the upper surface **306** by grinding or machining, such as at least one of laser machining, electrical discharge machining, or water jet machining. Examples of methods of using a laser to cut or machine a PCD table are disclosed in U.S. Pat. No. 9,062,505, the disclosure of which is incorporated herein, in its entirety, by this reference. In another example, the plurality of recessed features **308** may be formed in the upper surface **306** using acid etching, plasma etching, or other suitable etching techniques. Forming the plurality of recessed features **308** after leaching the PCD table **302** may result in a leached region that exhibits a first leach depth  $D_1$  and a second leach depth  $D_2$  that is less than the first leach depth  $D_1$  (FIG. 1B).

In another embodiment, the PCD table 302 may have the plurality of recessed features 308 formed in the upper surface 306 prior to leaching the PCD table 302. In such an embodiment, the plurality of recessed features 308 may be formed using any of the methods disclosed above. Additionally, the plurality of recessed features 308 may be formed using electrical discharge machining (e.g., wire electrical discharge machining) or pressed into the diamond particles before and/or during the HPHT process. The PCD table 302 including the plurality of recessed features 308 formed therein may then be leached using any of the leaching techniques disclosed herein. Forming the plurality of recessed features 308 prior to leaching the PCD table 302 may result in a leached region that exhibits a substantially uniform leach depth extending inwardly from the upper surface 306 and a base of each of the plurality of recessed features 308. For example, the leached region may be generally complementary to the topography of the outer surface of the top/upper surface of the PCD table 302 including surfaces formed by the recessed features 308.

In an embodiment, the plurality of recessed features 308 are formed in the upper surface 306 after leaching. For example, the plurality of recessed features 308 formed after leaching may be closer to a leach boundary-wear intersection location than if recessed features 308 were formed prior to leaching. As such, the plurality of recessed features 308 formed after leaching may exhibit a smaller average depth than the plurality of recessed features 308 formed prior to leaching.

Any of the recessed features disclosed herein may exhibit a number of suitable side, cross-sectional geometries. For example, any of the PCD tables disclosed herein may include a first plurality of recessed features that exhibits a first cross-sectional geometry (in side view) and a second plurality of recessed features that exhibits a second cross-sectional geometry (in side view) that is different than the first cross-sectional geometry. In another example, any of the PCD table disclosed herein may include a plurality of recessed features that each exhibits a substantially similar cross-sectional geometry. FIGS. 4A-4C are partial, side, cross-sectional of PCD tables that include at least one recessed feature formed therein that each exhibit different cross-sectional geometries, according to different embodiments. The PCD tables illustrated in FIGS. 4A-4C may be substantially the same as or similar to the PCD tables 102, 202, 302 (FIGS. 1A-3). Similarly, the cross-sectional geometries (in side view) of the recessed features illustrated in FIGS. 4A-4C may be used in any of the embodiments disclosed herein.

Referring to FIG. 4A, a PCD table 402a includes a leached region 418a and an unleached region 416a. The leached region 418a extends inwardly from an upper surface 406a of the PCD table 402a. The PCD table 402a also includes at least one recessed feature 408a formed in and extending inwardly from the upper surface 406a.

In the illustrated embodiment, the at least one recessed feature 408a exhibits a generally rectangular cross-sectional geometry (in side view). The generally rectangular cross-sectional geometry of the at least one recessed feature 408a may include a base 426a having a length and at least two side surfaces 434a extending from the base 426a to the upper surface 406a. The at least two side surfaces 434a may be substantially parallel, slightly diverge, or slightly converge relative to each other. In an embodiment, the at least two side surfaces 434a may also extend substantially perpendicularly or at an oblique angle relative to the upper surface 406a and/or the base 426a.

The generally rectangular cross-sectional geometry of the at least one recessed feature 408a may also include at least two corners 436a where the at least two side surfaces 434a meet the base 426a. The corners 436a may exhibit a radius of curvature, a fillet, or any other geometry. For example, at least one of the corners 436a may exhibit a relatively small radius of curvature when the corner 436a is sharp or exhibit a relatively large radius of curvature when the corner 436a is rounded. The radius of curvature of the corners 436a may correspond to a stress concentration factor exhibited by the corners. For example, a corner 436a that is sharp is expected to exhibit a relatively larger stress concentration factor than a corner 436a that is rounded. As such, a corner 436a may exhibit a sharp corner when the at least one recessed feature 408a is spaced relatively far from a leach boundary-wear intersection location. In an embodiment, the at least one recessed feature 408a may include a first corner that is relatively sharp and a second corner that is relatively round. In another embodiment, the at least one recessed feature 408a may only exhibit a relatively sharp corner along a selected length of the at least one recessed feature 408a.

Referring to FIG. 4B, a PCD table 402b includes a leached region 418b and an unleached region 416b. The leached region 418b extends inwardly from an upper surface 406b of the PCD table 402b. The PCD table 402b also includes at least one recessed feature 408b formed in and extending inwardly from the upper surface 406b.

The at least one recessed feature 408b exhibits a cross-sectional geometry (in side view) that is generally v-shaped. The generally v-shaped cross-sectional geometry may include at least two side walls 434b that extend and diverge from a base 426b to the upper surface 406b. At least one of the two side walls 434b may exhibit an oblique angle relative to the upper surface 406b. In the illustrated embodiment, the base 426b of the at least one recessed feature 408b exhibits a corner 436b. Similar to the at least two corners 436a (FIG. 4A), the corner 436b may be sharp or rounded. For example, the corner 436b may be sharp if the corner 436b is relatively spaced from a leach boundary-wear intersection location.

Referring to FIG. 4C, the PCD table 402c includes a leached region 418c and an unleached region 416c. The leached region 418c extends inwardly from an upper surface 406c of the PCD table 402c. The PCD table 402c also includes at least one recessed feature 408c formed in and extending inwardly from the upper surface 406c.

The at least one recessed feature 408c exhibits a cross-sectional geometry (in side view) that is arcuate (e.g., generally partially elliptical, such as partially circular). As such, the at least one recessed feature 408c may include a single continuous wall 434c that exhibits a generally concave shape relative to the upper surface 406c. Since the at least one recessed feature 408c does not include any corners, the at least one recessed feature 408c may exhibits a relatively low stress concentration factor. However, cracks formed in the PCD table 402c may be preferentially attracted to the at least one recessed feature 408c at least partially due to a proximity of the at least one recessed feature 408c to the crack.

Any of the recessed features disclosed herein (e.g., grooves, recesses, notches, dimples, channels, or networks) may exhibit any suitable pattern or network when formed in an upper surface of a PCD table. FIGS. 5-10E are top plan views of different PCD tables that exhibit different patterns of the plurality of recessed features formed in an upper surface thereof, according to different embodiments. The PCD tables illustrated in FIGS. 5-10E may be substantially

the same as or similar to the PCD tables 102, 202, 302, 402a-c (FIGS. 1-4C). For example, the PCD tables may be a partially leached PCD table that is bonded to a substrate. Any of the patterns illustrated in FIGS. 5-10E may be used in any of the embodiments disclosed herein. Additionally, any one or more of the patterns illustrated in FIGS. 5-10E or portions thereof may be combined together, without limitation.

Referring to FIG. 5, a PCD table 502 includes a plurality of recessed features 508 formed in an upper surface 506 thereof. The plurality of recessed features 508 form a generally triangular shape that is centered about a location on the upper surface 506 (e.g., a center of the upper surface 506). However, the plurality of recessed features 508 may form any other suitable shape, such as a generally circular shape, a generally rectangular shape, a generally pentagonal shape, a generally hexagonal shape, a generally elliptical shape, a generally crescent shape, or any other suitable shape. In the illustrated embodiment, the plurality of recessed features 508 only form a plane figure shape. However, the plurality of recessed features 508 may form a plurality of shapes that are each oriented differently (e.g., rotated, centered about a different location), exhibit different sizes, exhibit different shapes, intersect each other, or combinations thereof.

In the illustrated embodiment, the plurality of recessed features 508 extend from and contact an outer edge of the upper surface 506. As such, the plurality of recessed features 508 form four cells 528. Three of the cells 528 are formed along the outer edge of the upper surface 506 and form three distinct cutting surfaces. The plurality of recessed features 508 may limit spalling of one of the cells 528 from significantly adversely affecting the other cells 528. Additionally, the four cells 528 may limit spalling in a radial direction more than in a circumferential direction. Other patterns may form more or less cells and increase or decrease the amount of spalling in a radial and/or circumferential direction.

Referring to FIG. 6, a PCD table 602 includes a plurality of recessed features 608 formed in an upper surface 606 thereof. The plurality of recessed features 608 may extend radially from and/or relative to a location on the upper surface 606 (e.g., a center of the upper surface 606) to form a generally spoke-like pattern. As such, the plurality of recessed features 608 may form a plurality of cells 628 that may limit spalling along a circumferential direction. In an embodiment, the plurality of recessed features 608 may be substantially straight, curved, exhibit an "S" shape, or any other suitable shape. In an embodiment, each of the plurality of recessed features 608 may be angularly equidistantly spaced from each other. In another embodiment, at least some of the plurality of recessed features 608 may not be angularly equidistantly spaced from each other. In an embodiment, an angular spacing between two adjacent recessed features 608 may be equal to or greater than an angular spacing of an expected wear front in the PCD table 602 when the PCD table 602 is expected to spall.

FIGS. 7A-7D illustrate different embodiments in which a plurality of recessed features form different grid-like patterns in a PCD table. The grid-like patterns illustrated in FIGS. 7A-7D may substantially equally limit spalling of the PCD table in a circumferential and radial direction. Referring to FIG. 7A, a PCD table 702a may include a plurality of recessed features 708a formed in an upper surface 706a thereof. The plurality of recessed features 708a includes a plurality of first recessed features 708a' that extend substantially parallel to each other and a plurality of second recessed features 708a" that extend substantially parallel to each

other and substantially orthogonally relative to the plurality of first recessed features 708a'. As such, the plurality of recessed features 708a form a plurality of generally rectangular cells 728a that form a generally rectangular grid-like pattern. However, in an embodiment, the plurality of first and second recessed features 708a', 708a" extend obliquely relative to each other.

Referring to FIG. 7B, a PCD table 702b may include a plurality of recessed features 708b formed in an upper surface 706b thereof. The plurality of recessed features 708b includes plurality of first recessed features 708b' that extend substantially parallel to each other, a plurality of second recessed features 708b" that extend substantially parallel to each other, and a plurality of third recessed features 708b''' that extend substantially parallel to each other. In an embodiment, each of the plurality of first, second, and third recessed features 708b', 708b", 708b''' may extend obliquely relative to each other. In another embodiment, two of the plurality of first, second, or third recessed features 708b', 708b", 708b''' may extend substantially orthogonally relative to each other. In an embodiment, the plurality of recessed features 708b may form a plurality of generally triangular cells 728b that form a generally triangular grid-like pattern.

Referring to FIG. 7C, a PCD table 702c may include a plurality of recessed features 708c formed in an upper surface 706c thereof. The plurality of recessed features 708c form a plurality of generally hexagonal cells 728c that form a grid-like pattern.

Referring to FIG. 7D, a PCD table 702d may include a plurality of recessed features 708d formed in an upper surface 706d thereof. At least some of the plurality of recessed features 708d may be curved. In the illustrated embodiment, each of the plurality of recessed features 708d extend from at least two locations (e.g., eight locations) positioned at or near an outer edge of the upper surface 706d. The plurality of recessed features 708d may extend between generally opposite locations in substantially the same manner as longitudinal lines on an equatorial Robinson projection, an equatorial Winkel tripel projection, an equatorial azimuthal equidistant projection, an equatorial stereographic projection, an equal-area Mollweide projection, etc. As such, a concentration of the plurality of recessed features 708d may be greatest at or near the at least two locations. Additionally, the concentration of the plurality of recessed features 708d may be greater at and near the edge of the upper surface 706d than at a center of the upper surface 706d.

FIGS. 8A-8C illustrate different embodiments in which a plurality of recessed features form a generally two-dimensional or three-dimensional spiral pattern. The generally spiral pattern of the plurality of recessed features may limit spalling of the PCD table in a circumferential and radial direction. Referring to FIG. 8A, a PCD table 802a may include a plurality of recessed features 808a formed in an upper surface 806a thereof. The plurality of recessed features 808a may extend in a spiral from and/or relative to a location or area on the upper surface 806a (e.g., a center of the upper surface 806a). In an embodiment, each of the plurality of recessed features 808a may be equidistantly spaced from each other. In another embodiment, at least some of the plurality of recessed features 808a may not be equidistantly spaced from each other. In an embodiment, a circumferential spacing between two adjacent recessed features 808a may be equal to or greater than a circumferential width of an expected wear front in the PCD table 802a when the PCD table 802a is expected to spall.

Referring to FIG. 8B, a PCD table 802b may include a plurality of recessed features 808b formed in an upper surface 806b thereof. The plurality of recessed features 808b may include a plurality of first recessed features 808b' and a plurality of second recessed features 808b''. The plurality of first recessed features 808b' may be substantially the same as or similar to the plurality of recessed features 808a (FIG. 8A). For example, the plurality of first recessed features 808b' may extend along a spiral from a location or area on the upper surface 806b. The plurality of second recessed features 808b'' may extend between at least some of the plurality of first recessed features 808b' (e.g., generally crosswise or transverse to the first recessed features 808b'). As such, the plurality of second recessed features 808b'' may further limit the spalling in a circumferential and radial direction compared to the plurality of recessed features 808a (FIG. 8A).

Referring to FIG. 8C, a PCD table 802c may include a plurality of recessed features 808c formed in an upper surface 806c thereof. The plurality of recessed features 808c may extend along a spiral from a location or area on the upper surface 806c (e.g., a center of the upper surface 806c). However, the plurality of recessed features 808c may be relatively angular and/or discontinuous. The plurality of recessed features 808c may also include a plurality of recessed features that extend between the plurality of recessed features 808c.

FIGS. 8D-8I illustrate different PCD tables 802d-i that include a plurality of recessed features 808d-i formed in an upper surface 806d-i thereof. The plurality of recessed features 808d-i shown in FIGS. 8D-8I are embodiments of different spiral patterns that the plurality of recessed features 808d-i may form. Additionally, each of the plurality of recessed features 808d-i may be discontinuous recessed features (e.g., formed from a plurality of notches, dimples, recesses, or divots). In an embodiment, at least some of the plurality of recessed features 808d-i may be formed sufficiently close together that the at least some of the plurality of recessed features 808d-i forms a continuous feature (e.g., the plurality of recessed features 800d, 808g-i of FIGS. 8D, 8G-8I). In another embodiment, the plurality of notches may be uniformly distributed across the upper surface (e.g., the plurality of recessed features 808f of FIG. 8F). It is noted that any of the recessed features disclosed herein may be formed from a plurality of notches, dimples, recesses, or divots. It is also noted that any of the spiral patterns shown in FIGS. 8D-8I may be at least partially formed (e.g., completely formed) from a continuous channel instead of the plurality of notches, dimples, recesses, or divots. In some embodiments, a plurality of recessed features may include at least one substantially continuous recessed feature (e.g., at least one groove, at least one channel, etc.) and at least one discrete recessed feature (e.g., at least one notch, dimple, recess, or divot).

FIGS. 9A-9D illustrate different embodiments in which a plurality of recessed features form a plurality of generally concentric shapes that may limit spalling in at least a radial direction. Referring to FIG. 9A, a PCD table 902a may include a plurality of recessed features 908a formed in an upper surface 906a thereof. The plurality of recessed features 908a may form a plurality of generally rectangular shapes that are generally concentric relative to a location on the upper surface 906a such as a center of the upper surface 906a. The generally rectangular shapes formed by the plurality of recessed features 908a may form a plurality of cells 928a, four of which are adjacent to an outer edge of the upper surface 906a. The four cells 928a may partially define

four distinct cutting surfaces that may each spall without substantially adversely affecting the others. In operation, the outermost generally rectangular shape may be configured to limit spalling in a direction generally radially inwardly. However, the other generally rectangular shapes spaced inwardly from the outermost generally rectangular shape may be configured to further limit spalling in a general radial direction if the spalling extends past the outermost generally rectangular shape.

The plurality of recessed features 908a may form any suitable shapes (e.g., generally geometrically expanding or contracting shapes centered about a common point). For example, the plurality of recessed features 908a may form a generally circular shape, a generally rectangular shape, a generally pentagonal shape, a generally hexagonal shape, a generally elliptical shape, a generally crescent shape, or any other suitable shape. In an embodiment, the plurality of recessed features 908a may form a plurality of different shapes that are generally centered about a common point relative to each other. For example, the plurality of recessed features 908a may form an outermost shape that is generally rectangular and another shape that is inwardly generally centered relative to the outermost shape that is generally triangular. In an embodiment, at least one of the generally rectangular shapes may be rotated relative to the outermost generally rectangular shape.

Referring to FIG. 9B, a PCD table 902b includes a plurality of recessed features 908b formed in an upper surface 906b thereof. The plurality of recessed features 908b may include a plurality of first recessed features 908b' and a plurality of second recessed features 908b''. The plurality of first recessed features 908b' may form a plurality of shapes centered about a common point, such as a plurality of concentric generally circular shapes. The plurality of first recessed features 908b' may be generally concentric relative to a location on the upper surface 906b (e.g., a center of the upper surface 906b). The plurality of second recessed features 908b'' may be substantially the same as or similar to the plurality of recessed features 608 (FIG. 6). For example, the plurality of second recessed features 908b'' may extend from the same common point on the upper surface 906b that the plurality of first recessed features 908b' are centered about or extend from another location on the upper surface 906b.

The plurality of recessed features 908b illustrate an example of combining two of the patterns disclosed herein to form a single pattern. As such, the plurality of recessed features 908b may exhibit the benefits of the pattern discussed in FIG. 6 and the generally concentric shapes discussed in FIG. 9A. For example, the plurality of first recessed features 908b' may limit spalling in a radial direction while the plurality of second recessed features 908b'' may limit spalling in a circumferential direction.

In an embodiment, the plurality of first recessed features 908b' may not include a plurality of generally commonly centered shapes. Instead, the plurality of first recessed features 908b' may include a plurality of linear, convexly curved, and/or concavely recessed features that extend between the plurality of second recessed features 908b'' in any suitable manner. For example, the plurality of first recessed features 908b' may form a plurality of shapes that are not generally centered with respect to each other. In another example, at least some of the plurality of first recessed features 908b' may be radially offset from a circumferentially adjacent first recessed feature 908b' (e.g., at least some of the plurality of first recessed features 908b' may not form continuous shapes).

Referring to FIG. 9C, a PCD table 902c includes a plurality of recessed features 908c formed in an upper surface 906c thereof. The plurality of recessed features 908c include a plurality of first recessed features 908c', a plurality of second recessed features 908c'', and a plurality of third recessed features 908c'''. The plurality of first recessed features 908c' may be substantially similar to the plurality of recessed features 908a (FIG. 9A). For example, the plurality of first recessed features 908c' may include a plurality of generally commonly centered shapes, such as a plurality of concentric generally rectangular shapes. The outermost concentric generally rectangular shape may define four cells 928c adjacent to an outer edge of the upper surface 906c. The plurality of second recessed features 908c'' may include a plurality of generally concentric shapes that are different than the plurality of first recessed features 908c'. For example, the plurality of second recessed features 908c'' may be a plurality of concentric generally circular shapes. The plurality of second recessed features 908c''' may be positioned between the shapes formed by the plurality of first recessed features 908c'. Finally, the plurality of third recessed features 908c'''' form a plurality of radially-extending recessed features (e.g., a generally spoke-like pattern) that extend from a common location on the upper surface 906c.

The plurality of recessed features 908c'-908c'''' illustrate an example of combining three patterns to form a single network or pattern. For example, the plurality of first recessed features 908c' may limit spalling in a generally radial direction and the plurality of third recessed features 908c'''' may limit spalling in a generally circumferential direction. The plurality of first, second, and third recessed features 908c', 908c'', 908c'''' may form further spall-limiting features.

Referring to FIG. 9D, a PCD table 902d includes a plurality of recessed features 908d formed in an upper surface 906d thereof. The plurality of recessed features 908d may include a plurality of first recessed features 908d' and a plurality of second recessed features 908d''. The plurality of first recessed features 908d' may be substantially similar to the plurality of recessed features 708d (FIG. 7D). For example, the plurality of first recessed features 908d' may include a plurality of curved recessed features extending between two locations (e.g., end locations 909 and 911). The plurality of second recessed features 908d'' may form a plurality of generally concentric shapes, such as a plurality of generally concentric arcs that are generally centered about a common location (e.g., end locations 909, 911, a location on the upper surface 906d or a location off the upper surface 906d). For example, the location may be at one of the two locations that the plurality of first recessed features 908d' extend from and/or between. The plurality of first and second recessed features 908d', 908d'' may form a pattern exhibiting a higher concentration of recessed features near the outer edge of the upper surface 906d than relative to a concentration of recessed features near center of the upper surface 906d. Additionally, the plurality of first and second recessed features 908d', 908d'' form a pattern exhibiting a higher concentration of recessed features near the end locations 909 and 911. As such, the plurality of first and second recessed features 908d', 908d'' may limit spalling to a greater extent near the end locations 909, 911 than near the center of the upper surface 906d.

FIGS. 10A-10E illustrate different embodiments where a plurality of recessed features form a generally hypocycloid or hypotrochoid pattern. FIG. 10A illustrates a PCD table 1002a that includes a plurality of recessed features 1008a

formed in an upper surface 1006a thereof. The plurality of recessed features 1008a may include a plurality of generally arcuately-extending concavely or convexly curved recessed features (e.g., extending between cusps thereof) that, optionally, at least intersect with another recessed feature to form a cusp. In an embodiment, at least some of the plurality of recessed features 1008a may exhibit a different distance between the cusps thereof, a different radius of curvature, and/or a different length. In an embodiment, the plurality of recessed features 1008a may be substantially the same and form a hypocycloid or a hypotrochoid. For example, in the illustrated embodiment, the plurality of recessed features 1008a form a generally hypocycloid shape. However, in other embodiments, the plurality of recessed features 1008a form a generally hypotrochoid shape, a generally epicycloid shape, a generally epitrochoid shape, another suitable cycloid, or another suitable trochoid. During operation, the plurality of recessed features 1008a may limit spalling in a radial direction and a circumferential direction.

In an embodiment, the plurality of recessed features 1008a may form a shape (e.g., cycloid or trochoid) having at least 3 cusps, such as 4, 5, 5-10, 10-15, 15-20, or greater than 20 cusps. The number of cusps of the shape formed from the plurality of recessed features 1008a may correspond to the number of cells 1028a formed radially outwardly from the shape. In an embodiment, the plurality of recessed features 1008a may optionally intersect at the cusps thereof or the plurality of recessed features 1008a may optionally intersect at the cusps thereof and at one or more locations between the cusps thereof.

Referring to FIG. 10B, a PCD table 1002b includes a plurality of recessed features 1008b formed in an upper surface 1006b thereof. As shown in FIG. 10B, the plurality of recessed features 1008b include a plurality of generally arcuately-extending curved recessed features that intersect at cusps thereof. Similar to the plurality of recessed features 1008a (FIG. 10A), at least some of the plurality of recessed features 1008b may form one or more hypocycloids, hypotrochoids, or another suitable shape. The cusps of at least some of the plurality of recessed features 1008b may contact one or more radially inwardly or outwardly adjacent recessed features 1008b. As such, the plurality of recessed features 1008b may form a generally scale-like pattern (e.g., a plurality of contiguous hypocycloids). FIG. 10C also illustrates a plurality of recessed features 1008c formed in an upper surface 1006c of PCD table 1002c that include a plurality of generally extending curved recessed features that intersect at cusps thereof. The plurality of recessed features 1008c may form a plurality of generally concentric shapes (e.g., cycloids and/or trochoids). However, in some embodiments, the plurality of generally concentric shapes may not contact a radially adjacent recessed feature 1008c.

Referring to FIG. 10D, a PCD table 1002d includes a plurality of recessed features 1008d formed in an upper surface 1006d thereof. The plurality of recessed features 1008d may form a plurality of first recessed features 1008d' and a plurality of second recessed features 1008d''. The plurality of first recessed features 1008d' may be substantially similar to the plurality of recessed features 1008a (FIG. 10B). For example, the plurality of first recessed features 1008d' may include a plurality recessed features that intersect at the cusps thereof and contact one or more radially adjacent recessed features 1008d'. The plurality of second recessed features 1008d'' may be substantially similar to the plurality of recessed features 608 (FIG. 6). For example, the plurality of second recessed features 1008d'' may form a generally spoke-like pattern. As such, the

plurality of second recessed features **1008d"** may further limit spalling in a circumferential direction compared to the plurality of recessed features **1008b** (FIG. 10B).

Referring to FIG. 10E, a PCD table **1002e** includes a plurality of recessed features **1008e** formed in an upper surface **1006e** thereof. The plurality of recessed features **1008e** include a plurality of first recessed features **1008e'** and a plurality of second recessed features **1008e"**. The plurality of first recessed features **1008e'** may be substantially similar to the plurality of recessed features **1008c** (FIG. 10C). For example, the plurality of first recessed features **1008e'** may include a plurality of generally arcuately-extending curved recessed features that intersect at the cusps thereof. The plurality of first recessed features **1008e'** may form a plurality of generally commonly-centered shapes (e.g., cycloids and/or trochoids). The plurality of second recessed features **1008e"** may be substantially similar to the plurality of second recessed features **1008d"** (FIG. 10D). As such, the plurality of recessed features **1008e** may form a generally web-like pattern. The plurality of first recessed features **1008e'** may limit spalling generally in a radial direction and the plurality of second recessed features **1008e"** may limit spalling generally in a circumferential direction.

In an embodiment, the plurality of first recessed features **1008e'** may not form a plurality of generally concentric shapes. Instead, the plurality of first recessed features **1008e'** may include a plurality of curved recessed features that extend between the plurality of second recessed features **1008e"**. For example, at least some of the plurality of first recessed features **1008e'** may not intersect at the cusp thereof and may be radially spaced relative to a circumferentially adjacent first recessed feature **1008e'**.

The following working examples of the present disclosure set forth various configurations that have been used to form the PDC cutting elements disclosed herein. The following working examples provide further detail in connection with the embodiments described above.

#### Comparative Example 1

A conventional PDC was formed from a bimodal mixture of diamond particles having respective modes at about 30  $\mu\text{m}$  and about 2  $\mu\text{m}$ . The mixture of diamond particles was positioned adjacent to a cobalt-cemented tungsten carbide substrate. The plurality of diamond particles were sintered and bonded to the substrate in an HPHT process having a cell pressure of about 7.8 GPa and a temperature of about 1360° C. to form the conventional PDC including a PCD table. The PDC table was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . The conventional PDC did not have any recessed features formed in an upper surface thereof.

The conventional PDC was then subjected to a milling spallation test in which the PDC was used to cut a Barre granite workpiece. The test parameters used for the milling test were a back rake angle for the PDC of about 20°, an in-feed for the PDC of about 50.8 cm/min, a rotary speed on the workpiece of about 3000 RPM, an indexing across the workpiece (e.g., in the Y direction) of about 7.62 cm, about 3-5 seconds (no more than 10 seconds) between cutting passes, and the size of the Barre granite workpiece was about 63.5 cm by about 48.3 cm. The PDCs were held in a cutting tool holder, with the substrate of the PDCs tested thermally insulated on its back side via an alumina disc and

along its circumference by a plurality of zirconia pins. The conventional PDC was subject to the milling test until the conventional PDC spalled. Spalling of the PDC was determined using a “burnout” method in which spalling was detected when at least one of the operator detected sparks, the operator noticed black marks on the Barre granite, a sharp rise in the detected temperature, or a slight change in the force measurements.

FIG. 11 is a photograph of the conventional PDC after the conventional PDC spalled. FIG. 11 illustrates that the spalled conventional PDC includes a spalled region that extended significantly into the PCD table in both a radial direction and a circumferential direction. Additionally, the PCD table included a plurality of cracks (e.g., microcracks) that extended from the spalled region into the PCD table.

#### Example 2

A PDC was formed as described in comparative example 1 prior to leaching. The PDC table of example 2 was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . A plurality of recessed features having an average depth of about 75  $\mu\text{m}$  was then formed in the upper surface of the PCD table of example 2 using a laser. The plurality of recessed features included a plurality of circumferentially-extending first recessed features and a plurality of radially-extending second recessed features that were substantially similar to the plurality of first recessed features **1008e'** and the plurality of second recessed features **1008e"** (FIG. 10E), respectively. The PDC of example 2 was then tested in a milling spallation test using the same test parameters as comparative example 1. The PDC of example 2 was tested until the PDC of example 2 spalled.

FIG. 12A is a photograph of the PDC of example 2 after the PDC of example 2 spalled. FIG. 12A illustrates that the spalled PDC of example 2 included a spalled region that was radially and circumferentially limited by the plurality of first and second recessed features, respectively. As such, the spalled region is partially defined by the plurality of first and second recessed features. Additionally, the inventors believe that the plurality of recessed features limited cracks extending from the spalled region into the PCD table of example 2. As such, the plurality of recessed features may increase the usability of the PDC of example 2. For example, the PDC of example 2 can be subjected to another milling test by rotating the PDC of example 2 such that a portion of the PCD table of example 2 that does not include the spalled region forms the cutting contact area.

#### Example 3

A PDC was formed as described in comparative example 55 1 prior to leaching. The PDC table of example 3 was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . A plurality of recessed features having an 60 average depth of about 75  $\mu\text{m}$  was then formed in the upper surface of the PCD table of example 3 using a laser. The plurality of recessed features included a plurality of arcuately-extending first recessed features and a plurality of generally radially-extending second recessed features (e.g., 65 substantially similar to the plurality of first recessed features **1008e'** and the plurality of second recessed features **1008e"** (FIG. 10E), respectively). The PDC of example 3 was then

tested in milling spallation test using the same test parameters as comparative example 1. The PDC of example 3 was tested until the PDC of example 3 spalled.

FIG. 12B is a photograph of the PDC of example 3 after the PDC of example 3 spalled. FIG. 12B illustrates that the spalled PDC of example 3 included a spalled region that was radially limited by the plurality of first recessed features. As such, the spalled region is partially defined by the plurality of first recessed features. Additionally, the inventors believe that the plurality of recessed features limited cracks extending from the spalled region into the PCD table of example 3. As such, the plurality of recessed features may increase the usability of the PDC of example 3. For example, the PDC of example 3 can be subjected to another milling test by rotating the PDC of example 3 such that a portion of the PCD table of example 3 that does not include the spalled region forms the cutting contact area.

#### Example 4

A PDC was formed as described in comparative example 1 prior to leaching. The PDC table of example 4 was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . A plurality of recessed features having an average depth of about 75  $\mu\text{m}$  was then formed in the upper surface of the PCD table of example 4 using a laser. The plurality of recessed features included a plurality of arcuately-extending first recessed features and a plurality of generally radially-extending second recessed features (e.g., substantially similar to the plurality of first recessed features 1008e' and the plurality of second recessed features 1008e" (FIG. 10E), respectively). The PDC of example 4 was then tested in milling spallation test using the same test parameters as comparative example 1. The PDC of example 4 was tested until the PDC of example 4 spalled.

FIG. 12C is a photograph of the PDC of example 4 after the PDC of example 4 spalled. FIG. 12C illustrates that the spalled PDC of example 4 included a spalled region that was radially and circumferentially limited by the plurality of first and second recessed features, respectively. As such, the spalled region is partially defined by the plurality of first and second recessed features. Additionally, it is believed by the inventors that the plurality of recessed features limited cracks extending from the spalled region into the PCD table of example 4. As such, the plurality of recessed features may increase the usability of the PDC of example 4. For example, the PDC of example 4 can be subjected to another milling test by rotating the PDC of example 4 such that a portion of the PCD table of example 4 that does not include the spalled region forms the cutting contact surface.

#### Example 5

A PDC was formed as described in comparative example 1 prior to leaching. The PDC table of example 5 was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . A plurality of recessed features having an average depth of about 75  $\mu\text{m}$  was then formed in the upper surface of the PCD table of example 5 using a laser. The plurality of recessed features included a plurality of arcuately-extending first recessed features and a plurality of generally radially-extending second recessed features (e.g., substantially similar to the plurality of first recessed features

908b' and the plurality of second recessed features 908b" (FIG. 9B), respectively). The PDC of example 5 was then tested in milling spallation test using the same test parameters as comparative example 1. The PDC of example 5 was tested in a milling test until the PDC of example 5 spalled.

FIG. 12D is a photograph of the PDC of example 5 after the PDC of example 5 spalled. FIG. 12D illustrates that the spalled PDC of example 5 included a spalled region that was radially and circumferentially limited by the plurality of first and second recessed features. As such, the spalled region is partially defined by the plurality of first and second recessed features. Additionally, the inventors believe that the plurality of recessed features limited cracks extending from the spalled region into the PCD table of example 5. As such, the plurality of recessed features may increase the usability of the PDC of example 5. For example, the PDC of example 5 can be subjected to another milling test by rotating the PDC of example 5 such that a portion of the PCD table of example 5 that does not include the spalled region forms the cutting contact surface.

#### Example 6

A PDC was formed as described in comparative example 1 prior to leaching. The PDC table of example 6 was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . A plurality of recessed features having an average depth of about 75  $\mu\text{m}$  was then formed in the upper surface of the PCD table of example 6 using a laser. The plurality of recessed features included a plurality of arcuately-extending first recessed features and a plurality of generally radially-extending second recessed features (e.g., substantially similar to the plurality of first recessed features 908b' and the plurality of second recessed features 908b" (FIG. 9B), respectively). The PDC of example 6 was then tested in milling spallation test using the same test parameters as comparative example 1. The PDC of example 6 was tested until the PDC of example 6 spalled.

FIG. 12E is a photograph of the PDC of example 6 after the PDC of example 6 spalled. FIG. 12E illustrates that the spalled PDC of example 6 includes a spalled region that was radially and circumferentially limited by the plurality of first and second recessed features, respectively. As such, the spalled region is partially defined by the plurality of first and second recessed features. FIG. 12E also illustrates how generally commonly centered shapes may limit spallation. Additionally, it is believed by the inventors that the plurality of recessed features limited cracks extending from the spalled region into the PCD table of example 6. As such, the plurality of recessed features may increase the usability of the PDC of example 6. For example, the PDC of example 6 can be subjected to another milling test by rotating the PDC of example 6 such that a portion of the PCD table of example 6 that does not include the spalled region forms the cutting contact surface.

#### Example 7

A PDC was formed as described in comparative example 1 prior to leaching. The PDC table of example 7 was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . A plurality of recessed features having an average depth of about 75  $\mu\text{m}$  was then formed in the upper

surface of the PCD table of example 7 using a laser. The plurality of recessed features formed a generally rectangular grid-like pattern (FIG. 7A). The PDC of example 7 was then tested in milling spallation test using the same test parameters as comparative example 1. The PDC of example 7 was tested until the PDC of example 7 spalled.

FIG. 12F is a photograph of the PDC of example 7 after the PDC of example 7 spalled. FIG. 12F illustrates that the spalled PDC of example 7 included a spalled region that was radially and circumferentially limited by the plurality of recessed features. As such, the spalled region is partially defined by the plurality of recessed features. Additionally, it is believed by the inventors that the plurality of recessed features limited cracks extending from the spalled region into the PCD table of example 7. As such, the plurality of recessed features may increase the usability of the PDC of example 7. For example, the PDC of example 7 can be subjected to another milling test by rotating the PDC of example 7 such that a portion of the PCD table of example 7 that does not include the spalled region forms the cutting contact surface.

#### Example 8

A PDC was formed as described in comparative example 1 prior to leaching. The PDC table of example 8 was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . A plurality of recessed features having an average depth of about 75  $\mu\text{m}$  was then formed in the upper surface of the PCD table of example 8 using a laser. The plurality of recessed features form a plurality of generally commonly centered hypocycloids (e.g., similar to the plurality of recessed features 1008b (FIG. 10B)). The PDC of example 8 was then tested in milling spallation test using the same test parameters as comparative example 1. The PDC of example 8 was tested until the PDC of example 8 spalled.

FIG. 12G is a photograph of the PDC of example 8 after the PDC of example 8 spalled. FIG. 12G illustrates that the spalled PDC of example 8 included a spalled region that was radially and circumferentially limited by the plurality of first and second recessed features, respectively. As such, the spalled region is partially defined by the plurality of first and second recessed features. The area of the spalled region measured about 19  $\text{mm}^2$ , which is about 9.4% of the area of the upper surface of the PDC of example 8. FIG. 12G also illustrates how generally concentric shapes may act as fail-safes to an outermost shape. Additionally, it is believed that the plurality of recessed features limited cracks extending from the spalled region into the PCD table of example 8. As such, the plurality of recessed features may increase the usability of the PDC of example 8. For example, the PDC of example 8 can be subjected to another milling test by rotating the PDC of example 8 such that a portion of the PCD table of example 8 that does not include the spalled region forms the cutting contact surface.

#### Example 9

A PDC was formed as described in comparative example 1 prior to leaching. The PDC table of example 9 was then partially leached to form a leached region having a first leach depth from an upper surface of the PCD table of about 490  $\mu\text{m}$ , a side leach depth of about 80  $\mu\text{m}$ , and a  $L_1^*$  value of about 200  $\mu\text{m}$ . A plurality of recessed features having an average depth of about 75  $\mu\text{m}$  was then formed in the upper

surface of the PCD table of example 9 using a laser. The plurality of recessed features included a plurality of spirally-extending first recessed features and a plurality of second recessed features extending between the plurality of first recessed features (e.g., similarly to the plurality of first recessed features 808b' and the plurality of second recessed features 808b" (FIG. 8B), respectively). The PDC of example 9 was then tested in milling spallation test using the same test parameters as comparative example 1. The PDC of example 9 was tested until the PDC of example 9 spalled.

The PDC of example 9 included a spalled region that was radially and circumferentially limited by the plurality of first and second recessed features, respectively. As such, the spalled region is partially defined by the plurality of first and second recessed features. Additionally, it is believed that the plurality of recessed features limited cracks extending from the spalled region into the PCD table of example 9. As such, the plurality of recessed features may increase the usability of the PDC of example 9. For example, the PDC of example 9 can be subjected to another milling test by rotating the PDC of example 9 such that a portion of the PCD table of example 9 that does not include the spalled region forms the cutting contact surface.

#### Probability of Failure of Comparative Example 1 and Working Examples 2, 7, 8 and 9

The thermal stability for several of the PDCs disclosed herein were measured by determining a distance that the PDCs cut in a mill test prior to failure. Four PDCs were formed according to the methods disclosed in each of comparative example 1 and working examples 2, 7, 8, and 9. Each of the PDCs were then subjected to a milling test in which the PDCs are used to cut the same Barre granite workpiece without any coolant (e.g., dry cutting of the Barre granite workpiece in air). The test parameters used for the milling test were the same as described above in comparative example 1. Failure is determined when the PDCs can no longer cut the workpiece (e.g., spall). Spalling of the PDC was determined using a "burnout" method where spalling was detected when at least one of the operator detected sparks, the operator noticed black marks on the Barre granite, a sharp rise in the detected temperature, or a slight change in the force measurements. The distance each PDC cut prior to failure was calculated by: (the width of the workpiece)  $\times$  (the number of complete passes)  $+$  (the distance cut on the last pass prior to failure).

FIG. 13 is a graph showing probability of failure of comparative example 1 and working examples 2, 7, 8, and 9 versus distance each PDC cut prior to failure. FIG. 13 illustrates that a probability of failure at relatively large distances cut for working examples 2, 7, 8, and 9 was superior to comparative example 1. For example, the graph illustrates that the comparative example 1 exhibited a probability of failure of about 0.1 at a distance cut of about 305 inches, a probability of failure of about 0.4 at a distance cut of about 310 inches, and a probability of failure of about 0.75 at a distance cut of about 315 inches. In contrast, the graph illustrates that at least some of the working examples exhibit a probability of failure less than about 0.1 at a distance cut of about 315 inches or greater (e.g., about 315 inches to about 325 inches, about 325 inches to about 350, about 350 inches or greater), a probability of failure less than about 0.4 at a distance cut of about 325 inches or greater (e.g., about 325 inches to about 350 inches, about 350 inches to about 375 inches, about 375 inches to about 400 inches, greater than 400 inches), a probability of failure less than

about 0.75 at a distance cut of about 340 inches or greater (e.g., about 350 inches to about 375 inches, about 375 inches to about 400 inches, about 400 inches to about 425 inches, about 425 inches or greater).

The disclosed PDC embodiments may be used in a number of different applications including, but not limited to, use in a rotary drill bit (FIGS. 14A and 14B), a thrust-bearing apparatus, a radial bearing apparatus, a mining rotary drill bit (e.g., a roof bolt drill bit), and a wire-drawing die. The various applications discussed above are merely some examples of applications in which the PDC embodiments may be used. Other applications are contemplated, such as employing the disclosed PDC embodiments in friction stir welding tools.

FIG. 14A is an isometric view and FIG. 14B is a top plan view of an embodiment of a rotary drill bit 1400 for use in subterranean drilling applications, such as oil and gas exploration. The rotary drill bit 1400 includes at least one PCD element and/or PDC configured according to any of the previously described PDC embodiments. The rotary drill bit 1400 comprises a bit body 1402 that includes radially and longitudinally extending blades 1404 with leading faces 1406, and a threaded pin connection 1408 for connecting the bit body 1402 to a drilling string. The bit body 1402 defines a leading end structure for drilling into a subterranean formation by rotation about a longitudinal axis and application of weight-on-bit. At least one PDC cutting element, configured according to any of the previously described PDC embodiments may be affixed to the bit body 1402.

With reference to FIG. 14B, a plurality of PDCs 1412 are secured to the blades 1404. For example, each PDC 1412 may include a PCD table 1414 bonded to a substrate 1416. More generally, the PDCs 1412 may comprise any PDC disclosed herein, without limitation. For example, the PCD table 1414 may include the plurality of recessed features 1415 formed in an upper surface thereof. In addition, if desired, in some embodiments, a number of the PDCs 1412 may be conventional in construction. Also, circumferentially adjacent blades 1404 define so-called junk slots 1418 therebetween, as known in the art. Additionally, the rotary drill bit 1400 may include a plurality of nozzle cavities 1420 for communicating drilling fluid from the interior of the rotary drill bit 1400 to the PDCs 1412.

In an embodiment, the plurality of PDCs 1412 may be secured to the blades 1404 using a brazing technique, a mechanical fastener, a high temperature adhesive, press-fitting, or another suitable technique. The rotary drill bit 1400 may then be used in one or more subterranean drilling operations until at least one of the plurality of PDCs 1412 spall ("spalled PDC"). Spalling of the PDCs 1412 may be detected by sudden changes in force exerted by the plurality of PDCs 1412 against a subterranean surface, visual inspection, audible cues, or combinations thereof, etc. After one or more PDCs 1412 spall, the spalled PDC 1412 may be removed from the rotary drill bit 1400. For example, if the spalled PDC 1412 is brazed to the rotary drill bit 1400, the spalled PDC 1412 may be heated sufficiently to melt at least some of the braze material. The spalled PDC 1412 may then be rotated relative to the rotary drill bit 1400 to position a portion of the spalled PDC 1412 that does not include a spalled region in a cutting position. The spalled PDC 1412 may then be secured to the rotary drill bit 1400 using any of the techniques previously disclosed. The rotary drill bit 1400 may then be used in subterranean drilling operations.

FIGS. 14A and 14B merely depict one embodiment of a rotary drill bit that employs at least one PDC fabricated and structured in accordance with the disclosed embodiments,

without limitation. The rotary drill bit 1400 is used to represent any number of earth-boring tools or drilling tools, including, for example, core bits, roller-cone bits, fixed-cutter bits, eccentric bits, bi-center bits, reamers, reamer wings, or any other downhole tool including superabrasive compacts, without limitation.

The PDCs disclosed herein may also be utilized in applications other than cutting technology. For example, the disclosed PDC embodiments may be used in wire dies, 10 bearings, artificial joints, inserts, cutting elements, and heat sinks. Thus, any of the PDCs disclosed herein may be employed in an article of manufacture including at least one superabrasive element or compact.

Thus, the embodiments of PDCs disclosed herein may be used in any apparatus or structure in which at least one conventional PDC is typically used. In one embodiment, a rotor and a stator, assembled to form a thrust-bearing apparatus, may each include one or more PDCs (e.g., PDC 100 of FIGS. 1A and 1B) configured according to any of the embodiments disclosed herein and may be operably assembled to a downhole drilling assembly. U.S. Pat. Nos. 4,410,054; 4,560,014; 5,364,192; 5,368,398; and 5,480,233, the disclosure of each of which is incorporated herein, in its entirety, by this reference, disclose subterranean drilling systems within which bearing apparatuses utilizing PDCs disclosed herein may be incorporated. The embodiments of PDCs disclosed herein may also form all or part of heat sinks, wire dies, bearing elements, cutting elements, cutting inserts (e.g., on a roller-cone-type drill bit), machining inserts, or any other article of manufacture as known in the art. Other examples of articles of manufacture that may use any of the PDCs disclosed herein are disclosed in U.S. Pat. Nos. 4,811,801; 4,274,900; 4,268,276; 4,468,138; 4,738,322; 4,913,247; 5,016,718; 5,092,687; 5,120,327; 5,135,061; 5,154,245; 5,460,233; 5,544,713; and 6,793,681, the disclosure of each of which is incorporated herein, in its entirety, by this reference. Examples of other articles of manufacture that the PDCs disclosed herein can be used in are disclosed in U.S. Provisional Patent Application No. 62/232,732; U.S. patent application Ser. Nos. 13/790,046, 14/273,360, 14/275,574, and 14/811,699.

While various aspects and embodiments have been disclosed herein, other aspects and embodiments are contemplated. The various aspects and embodiment disclosed herein are for purposes of illustration and are not intended to be limiting. Additionally, the words "including," "having," and variants thereof (e.g., "includes" and "has") as used herein, including the claims, shall be open ended and have the same meaning as the word "comprising" and variants thereof (e.g., "comprise" and "comprises").

What is claimed is:

1. A polycrystalline diamond compact, comprising:  
a substrate; and  
a polycrystalline diamond table bonded to the substrate, the polycrystalline diamond table including an interfacial surface bonded to the substrate, an upper surface spaced from the interfacial surface, and at least one lateral surface extending between the upper surface and the interfacial surface, the polycrystalline diamond table including a plurality of diamond grains bonded together defining a plurality of interstitial regions, the polycrystalline diamond table including:  
an unleached region bonded to the interfacial surface, the unleached region including at least one interstitial constituent disposed in at least a portion of the plurality of interstitial regions thereof;

## 31

a leached region extending inwardly from the upper surface and at least a portion of the at least one lateral surface, the leached region being at least partially depleted of the at least one interstitial constituent; a plurality of recessed features extending from the upper surface through a portion of the polycrystalline diamond table, wherein a majority of the plurality of recessed features do not extend into the unleached region; wherein the leached region exhibits a first leach depth measured from the upper surface and a second leach depth measured from a base of each of the plurality of recessed features that is less than the first leach depth; and wherein at least some of the plurality of recessed features exhibit an average maximum width and an average maximum depth, the average maximum depth is greater than or equal to the average maximum width.

2. The polycrystalline diamond compact of claim 1, wherein the second leach depth is about 1% to about 75% less than the first leach depth.

3. The polycrystalline diamond compact of claim 1, wherein a depth of at least some of the plurality of recessed features exhibit a depth measured from the upper surface to a base thereof that is different from at least some other of the plurality of recessed features.

4. The polycrystalline diamond compact of claim 1, wherein the first leach depth is about 200  $\mu\text{m}$  to about 900  $\mu\text{m}$ .

5. The polycrystalline diamond compact of claim 1, wherein a depth of at least some of the plurality of recessed features exhibits a depth measured from the upper surface to the base thereof that is about 50  $\mu\text{m}$  to about 500  $\mu\text{m}$ .

6. The polycrystalline diamond compact of claim 1, further comprising a plurality of cells at least partially defined by at least one of the plurality of recessed features, each of the plurality of cells exhibits an average surface area that is 5% of a total surface area of the upper surface or less.

7. The polycrystalline diamond compact of claim 1, wherein the plurality of recessed features includes at least two immediately adjacent recessed features, at least a portion of each of the at least two immediately adjacent recessed features are substantially parallel to each other and exhibit a distance therebetween that is about 650  $\mu\text{m}$  or less.

8. The polycrystalline diamond compact of claim 1, wherein the plurality of recessed features exhibit a generally arcuate cross-section in side view, a generally triangular cross-section in side view, or a generally rectangular cross-section in side view.

9. The polycrystalline diamond compact of claim 1, wherein at least some of the plurality of recessed features extend generally radially.

10. The polycrystalline diamond compact of claim 1, wherein at least some of the plurality of recessed features extend along a spiral path.

11. The polycrystalline diamond compact of claim 1, wherein at least some of the plurality of recessed features generally forms at least one of a hypocycloid, hypotrochoid, or a generally commonly-centered shape.

12. The polycrystalline diamond compact of claim 1, wherein the plurality of recessed features form a triangular grid-like pattern, a rectangular grid-like pattern, or a hexagonal grid-like pattern.

13. The polycrystalline diamond compact of claim 1, wherein the leached region exhibits an  $L_1^*$  value that is about 50  $\mu\text{m}$  to about 1200  $\mu\text{m}$ , the  $L_1^*$  value is a distance between an initial wear front and an interface between the

## 32

leached region and the unleached region, wherein the initial wear front is a plane extending at about 20° angle relative to the at least one lateral surface, wherein the distance is a shortest distance from the initial wear front to the interface between the leached region and the unleached region measured substantially perpendicularly relative to the initial wear front.

14. A rotary drill bit, comprising:  
a bit body configured to engage a subterranean formation; and

a plurality of polycrystalline diamond cutting elements affixed to the bit body, at least one of the polycrystalline diamond cutting elements including:

a substrate; and

a polycrystalline diamond table bonded to the substrate, the polycrystalline diamond table including an interfacial surface bonded to the substrate, an upper surface spaced from the interfacial surface, and at least one lateral surface extending between the upper surface and the interfacial surface, the polycrystalline diamond table including a plurality of diamond grains bonded together defining a plurality of interstitial regions, the polycrystalline diamond table including:

a plurality of recessed features extending from the upper surface through a portion of the polycrystalline diamond table;

an unleached region bonded to the interfacial surface, the unleached region including at least one interstitial constituent disposed in at least a portion of the plurality of interstitial regions thereof; a leached region extending inwardly from the upper surface and at least a portion of the at least one lateral surface, the leached region being at least partially depleted of the at least one interstitial constituent, wherein the leached region exhibits a first leach depth measured from the upper surface and a second leach depth measured from a base of each of the plurality of recessed features that is less than the first leach depth, and wherein a majority of the plurality of recessed features do not extend into the unleached region; and

wherein at least some of the plurality of recessed features exhibit an average maximum width and an average maximum depth, the average maximum depth is greater than or equal to the average maximum width.

15. A polycrystalline diamond compact, comprising:

a substrate; and

a polycrystalline diamond table bonded to the substrate, the polycrystalline diamond table including an interfacial surface bonded to the substrate, an upper surface spaced from the interfacial surface, and at least one lateral surface extending between the upper surface and the interfacial surface, the polycrystalline diamond table including a plurality of diamond grains bonded together defining a plurality of interstitial regions, the polycrystalline diamond table including:

an unleached region bonded to the interfacial surface, the unleached region including at least one interstitial constituent disposed in at least a portion of the plurality of interstitial regions thereof;

a leached region extending inwardly from the upper surface and at least a portion of the at least one lateral surface, the leached region being at least partially depleted of the at least one interstitial constituent; a plurality of recessed features extending from the upper surface through a portion of the polycrystalline

33

diamond table, the plurality of recessed features forming a plurality of cells;  
 wherein an initial spallation of the polycrystalline diamond table in response to a milling spallation test is about 10% or less of the area of the upper surface of the 5 polycrystalline diamond table; and  
 wherein the leached region exhibits a first leach depth measured from the upper surface and a second leach depth measured from a base of each of the plurality of recessed features that is less than the first leach depth; 10 and  
 wherein at least some of the plurality of recessed features exhibit an average maximum width and an average maximum depth, the average maximum depth is greater than or equal to the average maximum width. 15

**16.** A polycrystalline diamond compact, comprising:  
 a substrate; and  
 a polycrystalline diamond table bonded to the substrate, the polycrystalline diamond table including an interfacial surface bonded to the substrate, an upper surface spaced from the interfacial surface, and at least one lateral surface extending between the upper surface and the interfacial surface, the polycrystalline diamond table including a plurality of diamond grains bonded together defining a plurality of interstitial regions, the 20 polycrystalline diamond table including:

34

a plurality of recessed features extending from the upper surface through a portion of the polycrystalline diamond table;  
 wherein the polycrystalline diamond table exhibits a probability of failure less than about 0.4 at a distance cut of at least about 325 inches when tested in a milling spallation test;  
 an unleached region bonded to the interfacial surface, the unleached region including at least one interstitial constituent disposed in at least a portion of the plurality of interstitial regions thereof;  
 a leached region extending inwardly from the upper surface and at least a portion of the at least one lateral surface, the leached region being at least partially depleted of the at least one interstitial constituent; wherein the leached region exhibits a first leach depth measured from the upper surface and a second leach depth measured from a base of each of the plurality of recessed features that is less than the first leach depth; and  
 wherein at least some of the plurality of recessed features exhibit an average maximum width and an average maximum depth, the average maximum depth is greater than or equal to the average maximum width.

\* \* \* \* \*